

# United States Patent [19]

Landholm et al.

[11] 3,942,987

[45] Mar. 9, 1976

[54] **PHOTOGRAPHIC MATERIALS WITH  
BALLASTED, ALKALI CLEAVABLE AZO  
DYES**

[75] Inventors: **Richard A. Landholm; Jan R.  
Haase, both of Rochester, N.Y.;  
James J. Krutak, Sr., Kingsport,  
Tenn.**

[73] Assignee: **Eastman Kodak Company**

[22] Filed: **Feb. 5, 1974**

[21] Appl. No.: **439,789**

## Related U.S. Application Data

[63] Continuation-in-part of Ser. No. 331,727, Feb. 12,  
1973, abandoned.

[52] **U.S. Cl.** ..... 96/73; 96/3; 96/29 D;  
96/77; 96/99

[51] **Int. Cl. 2 .. G03C 3/00; G03C 1/40; G03C 1/76;  
G03C 1/10**

[58] **Field of Search** ..... 96/3, 29 D, 77, 99, 73

## References Cited

### UNITED STATES PATENTS

3,134,672 5/1964 Blout et al. ..... 96/3

|           |         |                      |        |
|-----------|---------|----------------------|--------|
| 3,222,169 | 12/1965 | Green et al. ....    | 96/96  |
| 3,227,552 | 1/1966  | Whitmore .....       | 96/3   |
| 3,236,645 | 2/1966  | Husek et al. ....    | 96/99  |
| 3,255,001 | 6/1966  | Blout et al. ....    | 96/99  |
| 3,443,940 | 5/1969  | Bloom et al. ....    | 96/3   |
| 3,698,897 | 10/1972 | Gompf et al. ....    | 96/3   |
| 3,709,690 | 1/1973  | Cohen et al. ....    | 96/114 |
| 3,725,062 | 4/1973  | Anderson et al. .... | 96/3   |
| 3,728,113 | 4/1973  | Becker et al. ....   | 96/3   |

*Primary Examiner*—David Klein  
*Assistant Examiner*—Richard L. Schilling  
*Attorney, Agent, or Firm*—Elliott Stern; Daniel B.  
Reece, III

[57]

## ABSTRACT

Azo dye-providing compounds and photographic materials containing such compounds are described. The present compounds, as a function of photographic processing under alkaline conditions, provide a dye substance having a mobility different than that of the compound.

**98 Claims, No Drawings**

**PHOTOGRAPHIC MATERIALS WITH  
BALLASTED, ALKALI CLEAVABLE AZO DYES**

This is a continuation-in-part application of U.S. Ser. No. 331,727, filed Feb. 12, 1973, now abandoned.

This invention relates to the art of photography and more particularly, to color diffusion transfer photography employing cyan dye-providing compounds.

Color diffusion transfer processes generally involve the use of a photographic element comprising a support, at least one silver halide emulsion layer and an image dye-providing material which is contained in or contiguous said layer. The image dye-providing material typically can be thought of as having the structure Car-Col wherein Col is a colorant such as a dye or a dye precursor and Car is an associated carrier or monitoring group which as a function of alkaline processing effects a substantial change in the diffusivity of at least the Col portion of the compound.

After exposure, a photographic element as described above is treated with an alkaline processing solution to effect imagewise discrimination in the element. As mentioned previously, the imagewise discrimination is generally brought about by the monitoring or carrier group which, in the presence of the alkaline processing solution, is responsible for a substantial change in the diffusivity of at least the dye portion of the dye-providing material. As is known in the art, the dye-providing material can be initially immobile or initially mobile in the processing solution. Upon alkaline processing of an initially immobile dye-providing material, a mobile dye can be released imagewise or the material can be imagewise rendered soluble and thus mobile. If the material is initially mobile, the processing solution typically renders the material insoluble (and thus immobile) in an imagewise fashion.

It is well known in the art to utilize image dye-providing materials in a photographic element wherein an imagewise exposed element can be contacted with an alkaline processing solution to effect an imagewise difference in mobility of at least a portion of the dye-providing material, i.e., to effect release of a dye or dye precursor, to render said compound insoluble or soluble. It is the particular carrier or monitoring group which determines what form the change in diffusivity (of at least the dye portion of the material) will take. In certain instances, an increase in solubility of a given compound can be accomplished by substantially reducing the molecular weight of the compound; see, for example, the disclosure of Gompf U.S. Pat. No. 3,698,897, issued Oct. 17, 1972, in Fleckenstein et al allowed Ser. No. 351,763, a continuation-in-part of Ser. No. 282,796, filed Aug. 22, 1972, entitled PHOTOGRAPHIC SYSTEMS, in Anderson et al Ser. No. U.S. Pat. No. 3,725,062, filed July 6, 1971, entitled COLOR DIFFUSION TRANSFER PROCESSES and others. Exemplary of systems wherein the dye-providing compound splits off a dye are those described in Whitmore U.S. Pat. No. 3,227,552, issued Jan. 4, 1966, and Bloom U.S. Pat. No. 3,443,940, issued May 13, 1969, and Canadian Pat. No. 602,607, issued Aug. 2, 1960. Similarly, Yutzy U.S. Pat. No. 2,756,142, issued July 24, 1956, U.S. Pat. No. 2,774,668, issued Dec. 18, 1956, and U.S. Pat. No. 2,983,606, issued May 9, 1961, describe photographic elements wherein a dye-providing compound is rendered immobile in an imagewise fashion.

All of these prior systems have utility; however, it is desired to provide new compounds which provide new dyes having especially advantageous properties, such as improved hue, diffusibility, mordantability and the like.

We have found a class of cyan, azo dye-providing compounds well suited for use in color diffusion transfer color elements. The dye-providing compounds, as a function of typical processing under alkaline conditions, provide a cyan-colored substance having a mobility different than that of the compound.

The objects of the present invention are achieved through the use, in color diffusion transfer elements, of a new class of cyan, azo dye-providing compounds as well as the dyes provided thereby. Typically, these compounds are utilized in a photosensitive element which comprises a support having thereon at least one photosensitive silver halide emulsion, and at least one of said layers having associated therewith a cyan, azo dye-providing compound of this invention.

The compounds of this invention can be represented by the following formulas:



or



wherein

Car represents a carrier moiety which, as a function of oxidation under alkaline conditions, provides a substance having a mobility different than that of said compound;

X represents a bivalent linking group of the formula  $-\text{R}^2-\text{L}_n-\text{R}^2-$  where each  $\text{R}^2$  can be the same or different and each represents an alkylene radical having 1 to about 8 carbon atoms; a phenylene radical; or a substituted phenylene radical having 6 to about 9 carbon atoms; L represents a bivalent radical selected from oxy, carbonyl, carboxamido, carbamoyl, sulfonamido, sulfamoyl, sulfinyl or sulfonyl; n is an integer having a value of 0 or 1; p is 1 when n equals 1 and p is 1 or 0 when n equals 0, provided that when p is 1 the carbon content of the sum of both  $\text{R}^2$  radicals does not exceed 14 carbon atoms;

R represents a hydrogen atom, or an alkyl radical having 1 to about 6 carbon atoms;

J represents a bivalent radical selected from sulfonyl or carbonyl;

m and q each represent an integer having a value of 0 or 1;

Q represents a hydrogen atom, a hydroxy radical, or a radical having the formula  $-\text{NHCOR}^3$  or  $-\text{NH}-\text{SO}_2\text{R}^3$  wherein  $\text{R}^3$  is an alkyl radical having 1 to about 6 carbon atoms, a substituted alkyl radical having 1 to

about 6 carbon atoms, benzyl, phenyl, or a substituted phenyl radical having 6 to about 9 carbon atoms;

G represents a hydroxy radical, a salt thereof, or a hydrolyzable acyloxy group having the formula:



wherein  $\text{R}^4$  is an alkyl radical having 1 to about 18 carbon atoms, phenyl or substituted phenyl having 6 to about 18 carbon atoms;

D represents a halogen atom, a cyano radical, a nitro radical, a trifluoromethyl radical, an alkyl radical having 1 to about 6 carbon atoms, an alkoxy radical having 1 to about 6 carbon atoms, a carboxy radical, a carboxylic acid ester having the formula  $-\text{COOR}^4$  wherein  $\text{R}^4$  is as described previously, a fluorosulfonyl radical, a  $-\text{SO}_3\text{-phenyl}$  radical or a substituted  $-\text{SO}_3\text{-phenyl}$  radical having 6 to about 9 carbon atoms, a sulfo radical, a sulfamoyl radical having the formula  $-\text{SO}_2\text{NR}^5\text{R}^6$  wherein  $\text{R}^5$  represents hydrogen or an alkyl group having 1 to about 6 carbon atoms and  $\text{R}^6$  represents hydrogen, an alkyl radical having 1 to about 6 carbon atoms, a substituted alkyl radical having 1 to about 6 carbon atoms, a benzyl radical, a phenyl radical, a substituted phenyl radical having 6 to about 9 carbon atoms, an alkyl carbonyl radical having 1 to about 8 carbon atoms, or a phenyl carbonyl radical having 6 to about 9 carbon atoms, with the proviso that the carbon content of the sum of  $\text{R}^5$  and  $\text{R}^6$  not exceed 14 carbon atoms; a carbamoyl radical having the formula  $-\text{CON}(\text{R}^5)_2$  wherein each  $\text{R}^5$  can be the same or different and is as described previously; an alkyl- or substituted alkylsulfonyl radical having 1 to about 8 carbon atoms, a phenyl- or substituted phenylsulfonyl radical having 6 to about 9 carbon atoms; or D can represent a substituent having the formula  $\text{CAR-}[\text{X-}(\text{NR-J})_q]_m-$  or  $\text{CAR-X-J-}$ , provided that the  $\text{CAR-}[\text{X-}(\text{NR-J})_q]_m-$  substituent on the naphthalene nucleus of Formula I is replaced by an M group or the  $\text{CAR-X-J-NH-}$  substituent on the naphthalene nucleus of Formula II is replaced by a Q group wherein Car, X, J, R, q and m are as described previously.

E represents a hydrogen atom, a halogen atom, a nitro radical, a cyano radical or a trifluoromethyl radical;

M represents a hydrogen atom, a carboxy radical, a carboxylic acid ester having the formula  $-\text{COOR}^4$  wherein  $\text{R}^4$  is as described previously, a sulfo radical, a sulfamoyl radical having the formula  $-\text{SO}_2\text{NR}^5\text{R}^6$ , a

carbamoyl radical having the formula  $-(\text{CON}(\text{R}^5)_2)$  wherein  $\text{R}^5$  and  $\text{R}^6$  are as described previously, an alkyl- or substituted alkylsulfonyl radical having 1 to about 8 carbon atoms, or a phenyl- or substituted phenylsulfonyl radical having 6 to about 9 carbon atoms;

with the proviso that there be no more than one sulfo radical and no more than one carboxy radical present in said compound.

As mentioned above, the present compounds contain a carrier moiety (Car-) which, as a function (direct or inverse) of oxidation under alkaline conditions, pro-

vides a substance having a mobility different than that of the starting compound. Depending upon the carrier used, the dye-providing compounds of this invention can be of two basic types: (1) initially immobile compounds of which at least a portion is rendered mobile or diffusible as a function of development, or (2) initially mobile or diffusible compounds which are rendered immobile as a function of development. Carriers useful in initially immobile dye-providing compounds such as those wherein the carrier, under alkaline conditions, effects a splitting off of a ballast group from the dye moiety are described further in Whitmore Canadian Pat. No. 602,607, dated Aug. 2, 1960, and Whitmore U.S. Pat. No. 3,227,552, issued Jan. 4, 1966, both incorporated herein by reference. Among the preferred initially immobile compounds are those in which the carrier, as a function of oxidation under alkaline conditions, releases a dye having a mobility different than that of the starting immobile compound. For example, useful carriers for compounds in which the carrier moiety undergoes intramolecular ring closure upon oxidation to split off a dye are described in U.S. Pat. Nos. 3,443,939, 3,443,940 and 3,443,941, all issued May 13, 1969, and all incorporated herein by reference. Special initially immobile carriers useful in forming a diffusible substance as an inverse function of oxidation are described in copending Hinshaw and Condit application Ser. No. 326,628, filed Jan. 26, 1973, and entitled "Positive-Working Immobile Photographic Compounds and Photographic Elements Containing Same," incorporated herein by reference. Improved initially immobile dye-providing compounds which undergo redox reactions followed by alkali cleavage of the carrier to split off a dye are disclosed in Fleckenstein et al Ser. No. 282,796, filed Aug. 22, 1972, now abandoned, entitled "Photographic Systems," incorporated herein by reference. The ballasted phenolic and naphtholic carriers of Fleckenstein et al are among preferred carrier moieties. Still other useful carriers are described in U.S. Pat. No. 3,628,952, issued Dec. 21, 1971. Additionally, carriers useful in the formation of initially mobile compounds such as those wherein the carrier functions as a developer are described in Friedman U.S. Pat. No. 2,543,691, issued Feb. 27, 1951; U.S. Pat. No. 2,983,606, issued May 8, 1961; and U.S. Pat. No. 3,255,001, issued June 7, 1966; all incorporated herein by reference. Carriers of this latter type include various hydroquinone moieties.

Examples of bivalent alkylene linking groups representative of  $\text{R}^2$  are  $-\text{CH}_2-$ ,  $-\text{C}_2\text{H}_4-$ ,  $-\text{C}_6\text{H}_{12}-$ ,  $-\text{C}_3\text{H}_6-$ ,  $-\text{C}_4\text{H}_8-$ , etc., as well as branched alkylene radicals such as



References hereinafter to *o*, *m* and *p* mean that either the ortho, meta or para radicals are indicated, as the case may be.

Examples of phenylene and substituted phenylene radicals representative of  $\text{R}^2$  are *o,m,p*-phenylene, *o,m,p*-phenylene substituted with chloro, methoxy, butoxy, bromo, cyano, nitro, methyl, ethyl, carboxy, sulfo, amino, etc.

As used herein the oxygen- or sulfur-containing bivalent radicals representative of L are oxy ( $-\text{O}-$ ), car-

bonyl ( $-\text{CO}-$ ), carboxamido ( $-\text{CONH}-$ ), carbamoyl ( $-\text{NHCO}-$ ), sulfonamido ( $-\text{SO}_2\text{NH}-$ ), sulfamoyl ( $-\text{NHSO}_2-$ ), sulfinyl ( $-\text{SO}-$ ) and sulfonyl ( $-\text{SO}_2-$ ). Therefore, non-limiting examples of bivalent linking groups which may be represented by X are



etc.

Examples of the groups which R may represent are hydrogen, methyl, ethyl, isopropyl, pentyl, hexyl, etc. The alkyl group represented by R may additionally be substituted with cyano, hydroxy, methoxy, etc.

Examples of groups representative of Q are a hydrogen atom, a hydroxy radical or a radical having the formula  $-\text{NHCOR}^3$  or  $-\text{NHSO}_2\text{R}^3$  wherein R<sup>3</sup> is as described previously such as  $-\text{NHCOCH}_3$ ,  $-\text{NHCOCH}_2\text{CH}_3$ ,  $-\text{NHCOCH}_2\text{CH}_2\text{CH}_3$ ,  $-\text{NHCOCH}_2\text{CH}_2\text{CN}$ ,  $-\text{NHCOCH}_2\text{CH}_2\text{SO}_2\text{NH}_2$ ,  $-\text{NHCOCH}_2\text{CH}_2\text{CH}_5$ ,  $-\text{NHCOCH}_2\text{CH}_2\text{COOH}$ ,  $-\text{NHSO}_2\text{CH}_3$ ,  $-\text{NHSO}_2\text{C}_6\text{H}_4\text{CN}$ ,  $-\text{NHSO}_2\text{C}_6\text{H}_4\text{Cl}$ ,  $-\text{NHSO}_2\text{C}_6\text{H}_5$ ,  $-\text{NHCOC}_6\text{H}_5\text{SO}_3\text{H}$ ,  $-\text{NHSO}_2\text{C}_6\text{H}_4\text{OCH}_3$ , etc.

Examples of the groups which G may represent are hydroxy, salts thereof such as alkali metal (e.g.,  $-\text{O}^-\text{Li}^+$ ,  $-\text{O}^-\text{K}^+$ ,  $-\text{O}^-\text{Na}^+$ ) salts and photographically inactive ammonium salts thereof such as  $-\text{O}^-\text{NH}_4$ ,  $-\text{O}^-\text{NH}(\text{CH}_3)_3$ ,  $-\text{O}^-\text{NH}(\text{C}_2\text{H}_5)_4$ ,



i.e., a trialkyl or tetralkyl ammonium salt (sometimes called "amine salts") which does not adversely affect the photographic utility of the cyan image dye-providing compound or the physical or chemical processes which occur during development of the image.

G may also advantageously represent a hydrolyzable acyloxy group having the formula



wherein R<sup>4</sup> is as described previously. Non-limiting examples of these hydrolyzable groups are



30

35



40



etc.

Examples of substituents which D may represent are chloro, bromo, fluoro, a cyano radical ( $-\text{CN}$ ), a nitro radical ( $-\text{NO}_2$ ), methyl, isopropyl, ethyl, butyl, hexyl, etc., methoxy, ethoxy, isopropoxy, hexyloxy, butoxy, a carboxylic acid ester such as  $-\text{COOCH}_3$ ,  $-\text{COOC}_1\text{H}_{23}$ ,  $-\text{COOC}_2\text{H}_5$ ,  $-\text{COOC}_6\text{H}_5$ ,



55 radical including salts thereof, such as alkali metal salts or photographically inactive ammonium salts (e.g.,  $-\text{COO}^-\text{Li}^+$ ,  $-\text{COO}^-\text{K}^+$ ,  $-\text{COO}^-\text{Na}^+$ ,  $-\text{COO}^-\text{NH}_4^+$ , etc.), a fluorosulfonyl radical ( $-\text{SO}_2\text{F}$ ), a  $-\text{SO}_3\text{C}_6\text{H}_5$  radical,



65

etc., a sulfo radical including salts thereof, such as alkali metal or photographically inactive ammonium salts (e.g.,  $-\text{SO}_3\text{H}$ ,  $-\text{SO}_3^-\text{Li}^+$ ,  $\text{SO}_3^-\text{K}^+$ ,  $-\text{SO}_3^-\text{Na}^+$ ,  $-\text{SO}_3^-\text{NH}_4^+$ , etc.);  $-\text{SO}_2\text{NH}_2$ ,  $-\text{SO}_2\text{NHCH}_3$ ,  $-\text{SO}_2\text{NHC}_2\text{H}_5$ ,  $-\text{SO}_2\text{N}(\text{CH}_3)_2$ ,  $-\text{SO}_2\text{NHCH}_2\text{C}_6\text{H}_5$ ,



5



15

$-\text{SO}_2\text{NHC}_2\text{H}_4\text{CN}$ ,  $-\text{SO}_2\text{NHCOC}_6\text{H}_5$ ,  $-\text{SO}_2\text{NHCOCH}_3$ ,  $-\text{SO}_2\text{NHCOC}_3\text{H}_7$ ,



20

$\text{SO}_2\text{NHCOCH}_2\text{C}_6\text{H}_5$ ,  $-\text{SO}_2\text{NHC}_2\text{H}_4\text{SO}_3\text{H}$ ,



etc.;  $-\text{CONH}_2$ ,  $-\text{CON}(\text{C}_2\text{H}_5)_2$ ,



$-\text{CONHCH}_3$ ,  $-\text{CONHC}_5\text{H}_{11}$ , etc.;  $-\text{SO}_2\text{CH}_3$ ,



$-\text{SO}_2\text{C}_6\text{H}_{13}$ ,  $-\text{SO}_2\text{C}_2\text{H}_4\text{CN}$ ,  $-\text{SO}_2\text{C}_6\text{H}_5$ ,

$-\text{SO}_2\bullet\text{O}\bullet-\text{COOH}$ ,  $-\text{SO}_2\bullet\text{O}\bullet-\text{SO}_2\text{F}$ ,  $-\text{SO}_2\text{C}_2\text{H}_4\text{OH}$ ,  $-\text{SO}_2\bullet\text{O}\bullet-\text{OCH}_3$ ,

$-\text{SO}_2(\text{CH}_2)_3\text{SO}_2\text{NH}_2$ ,  $-\text{SO}_2(\text{CH}_2)_3\text{SO}_3\text{H}$ , etc.

Examples of substituents which E may represent are hydrogen, chloro, bromo, fluoro, nitro, cyano or trifluoromethyl.

Examples of substituents which M may represent are hydrogen, carboxy,  $-\text{COOC}_{11}\text{H}_{23}$ ,  $-\text{COOCH}_3$ ,  $-\text{COOC}_6\text{H}_5$ ,



$-\text{COOC}_{12}\text{H}_{25}$ ,  $-\text{SO}_3\text{H}$ ,  $-\text{SO}_3^-\text{Li}^+$ ,  $-\text{SO}_3^-\text{Na}^+$ , etc.,  $-\text{SO}_2\text{NH}_2$ ,  $-\text{SO}_2\text{NHCH}_3$ ,  $-\text{SO}_2\text{NHC}_2\text{H}_5$ ,  $-\text{SO}_2\text{N}(\text{CH}_3)_2$ ,  $-\text{SO}_2\text{NHCH}_2\text{C}_6\text{H}_5$ ,



$-\text{SO}_2\text{NHC}_2\text{H}_4\text{SO}_2\text{NH}_2$ ,  $-\text{SO}_2\text{NHCOC}_6\text{H}_5$ ,  $-\text{SO}_2\text{NHCOCH}_3$ ,  $-\text{SO}_2\text{NHCOC}_3\text{H}_7$ ,



$-\text{SO}_2\text{NHCOCH}_2\text{C}_6\text{H}_5$ ,  $-\text{SO}_2\text{NHC}_2\text{H}_5\text{SO}_3\text{H}$ ,

15

etc.,  $-\text{CONH}_2$ ,  $-\text{CON}(\text{C}_2\text{H}_5)_2$ ,



20

$-\text{CONHCH}_3$ ,  $-\text{CONHC}_6\text{H}_5$ , etc.,  $-\text{SO}_2\text{CH}_3$ ,  $-\text{SO}_2\text{C}_2\text{H}_5$ ,



$-\text{SO}_2\text{C}_2\text{H}_4\text{CN}$ ,  $-\text{SO}_2\text{C}_3\text{H}_6\text{OH}$ ,

35



etc.

Preferred compounds are those having Formulas I and II above wherein:

Car represents a carrier moiety which, as a function of oxidation under alkaline conditions, releases a dye having a mobility different than that of said compound;

$\text{R}^2$  represents an alkylene radical having 1 to about 4 carbon atoms, phenylene or phenylene substituted with carboxy, chloro, methyl or methoxy;

L represents sulfamoyl, sulfonamido, carbamoyl or carboxamido;

R represents hydrogen;

$q$  is an integer having a value of 1;

$m$  is an integer having a value of 0 or 1;

Q represents hydrogen, hydroxy,  $-\text{NHCOR}^3$  or

$-\text{NHSO}_2\text{R}^3$  wherein  $\text{R}^3$  represents an alkyl radical having 1 to about 4 carbon atoms; an alkyl radical having 1 to about 4 carbon atoms substituted with hydroxy, cyano, sulfamoyl, carboxy or sulfo; benzyl, phenyl or phenyl substituted with carboxy, chloro, methyl, methoxy or sulfamoyl;

D represents chloro, fluoro, bromo, cyano, trifluoromethyl, nitro, fluorosulfonyl, alkylsulfonyl having 1 to about 6 carbon atoms, alkylsulfonyl having 1 to about 6 carbon atoms substituted with hydroxy, phenyl, cyano, sulfamoyl, carboxy, fluorosulfonyl or sulfo; phenylsulfonyl; phenylsulfonyl substituted with hydroxy, sulfamoyl, fluorosulfonyl, carboxy or sulfo; a sulfamoyl radical having the formula  $-\text{SO}_2\text{NHR}^6$  wherein  $\text{R}^6$  is hydrogen, an alkyl radical having 1 to about 4 carbon atoms, or an alkyl radical having 1 to

65

about 4 carbon atoms substituted with hydroxy, cyano, sulfamoyl, carboxy or sulfo; benzyl, phenyl or phenyl substituted with hydroxy, sulfonyl, sulfamoyl, carboxy or sulfo; a carbamoyl radical having the formula  $-\text{CON}(\text{R}^5)_2$  wherein  $\text{R}^5$  is hydrogen or methyl, and

D can represent a substituent having the formula  $\text{Car}[\text{X}-(\text{NR-J})_q]_m-$  or  $\text{Car-X-J-}$ , provided that the  $\text{Car}[\text{X}-(\text{NR-J})_q]_m-$  substituent on the naphthalene nucleus of Formula I is replaced by an M group or the  $\text{Car-X-J-NH-}$  substituent on the naphthalene nucleus of Formula II is replaced by a Q group wherein Car, X, J, R, q and m are as described previously;

E represents hydrogen, fluoro, or chloro; and

M represents hydrogen or a sulfamoyl radical of the formula  $-\text{SO}_2\text{NHR}^6$  wherein  $\text{R}^6$  is hydrogen; an alkyl radical of 1 to about 4 carbon atoms; an alkyl radical having 1 to about 6 carbon atoms substituted with hydroxy, cyano, sulfamoyl, carboxy, or sulfo; benzyl, phenyl or phenyl substituted with hydroxy, sulfamoyl, carboxy or sulfo.

Especially preferred compounds are those having Formulas I and II above wherein the  $\text{Car-X-J-NH-}$  substituent in Formula II is in the 5-position on the naphthalene nucleus relative to G; and the  $\text{Car}[\text{X}-(\text{NR-J})_q]_m-$  substituent in Formula I is in the 5- or 6-position on the naphthalene nucleus relative to G;

$\text{R}^2$  represents an alkylene radical having 1 to about 4 carbon atoms, or phenylene;

L represents sulfamoyl or sulfonamido;

J represents sulfonyl;

Q is in the 8-position relative to G and represents hydrogen, hydroxy,  $-\text{NHSO}_2\text{R}^3$  or  $-\text{NHCOC}_6\text{H}_4$ ;

G represents hydroxy, a photographically inactive ammonium salt thereof, or a hydrolyzable acyloxy group having the formula:



wherein  $\text{R}^4$  is an alkyl radical having 1 to about 18 carbon atoms, phenyl or phenyl substituted with chloro or nitro;

D represents chloro, bromo, cyano, trifluoromethyl, nitro, alkylsulfonyl having 1 to about 6 carbon atoms, or benzylsulfonyl;

E represents hydrogen; and

M represents hydrogen.

Even more preferred compounds are those wherein

X represents



G represents hydroxy or a hydrolyzable acyloxy group; and

D represents an alkylsulfonyl radical having 1 to about 4 carbon atoms.

Even more especially preferred compounds are those having Formulas I and II above wherein Car- represents a radical of the formula:

III.



wherein Ball represents an organic ballasting group of such size and configuration as to render the compound nondiffusible during development in the alkaline processing composition and Y represents the carbon atoms necessary to complete a benzene or naphthalene nucleus including substituted benzene or naphthalene. When Y represents the atom necessary to complete a naphthalene nucleus, Ball can be attached to either ring thereof. Preferred ballasting groups are those wherein -Ball represents



Examples of some preferred carriers are as follows:





The nature of the ballast group (Ball) in the Formula III for the compounds described above is not critical as long as it confers nondiffusibility to the compounds. Typical ballast groups include long straight or branched chain alkyl radicals linked directly or indirectly to the compound as well as aromatic radicals of the benzene and naphthalene series indirectly attached or fused directly to the benzene nucleus, etc. Useful ballast groups generally have at least 8 carbon atoms such as a substituted or unsubstituted alkyl group of 8 to 22 carbon atoms, an amide radical having 8 to 30 carbon atoms, a keto radical having 8 to 30 carbon atoms, etc., and may even comprise a polymer backbone. Especially preferred compounds are those wherein the ballast is attached to the benzene nucleus through a carbamoyl radical ( $-\text{NHCO}-$ ) or a sulfamoyl radical ( $-\text{SO}_2\text{NH}-$ ) in which the nitrogen is adjacent the ballast group.

In addition to the ballast, the benzene nucleus in the above formula may have groups or atoms attached thereto such as the halogens, alkyl, aryl, alkoxy, aryloxy, nitro, amino, alkylamino, arylamino, amido, cyano, alkylmercapto, keto, carboalkoxy, heterocyclic groups, etc.

In a preferred embodiment of this invention CAR is a moiety which as a function of oxidation under alkaline conditions, releases a dye having a mobility different than that of the image dye-providing compounds.

The preferred novel dyes which are released from the carrier moieties as a function of oxidation under alkaline conditions may be represented by the following formulas:



wherein

Z represents  $\text{NH}_2\text{SO}_2-$ ,  $\text{HSO}_2$  or lower alkyl-NH-; and X, R, J, q, m, O, G, M, D and E are as described previously, except that the Car substituents described for D are replaced by Z. The preferred released dyes, of course, correspond to the above mentioned preferred image dye-providing compounds set forth above.

When Z represents  $-\text{SO}_2\text{H}$ , the dyes thus represented may be released by the reactions described in Bloom, U.S. Pat. No. 3,443,940, in Puschel, U.S. Pat. No. 3,628,952 and Gompf, U.S. Pat. No. 3,698,897. When Z represents lower alkyl-NH- (i.e., an alkyl group having 1 to about 4 carbon atoms), the dyes thus represented may be released by the reactions described in Hinshaw et al., U.S. Ser. No. 326,628. The especially preferred released dyes of our invention are those represented by Formulas IV and V above when Z represents  $-\text{SO}_2\text{NH}_2$ . These dyes may be released by the reactions described in Fleckenstein et al allowed Ser. No. 351,763, a continuation-in-part of, U.S. Ser. No. 282,796 from the carrier moieties described by Formula III.

A suitable process for producing a photographic transfer image in color using the compounds of our invention, for example those wherein Car is as shown in Formula III, comprises the steps of:

1. treating the above-described photosensitive element with an alkaline processing composition in the presence of a silver halide developing agent to effect development of each of the exposed silver halide emulsion layers, thereby oxidizing the developing agent and the oxidized developing agent in turn cross-oxidizing the sulfonamido compound;
2. forming an imagewise distribution of diffusible released dye as a function of the imagewise exposure of each of the silver halide emulsion layers by cleaving each cross-oxidized sulfonamido compound; and
3. diffusing to a dye image-receiving layer at least a portion of each of the imagewise distributions of diffusible released dye to provide an image.

The photosensitive element in the above-described process can be treated with an alkaline processing composition to effect or initiate development in any manner. A preferred method for applying processing composition is by use of a rupturable container or pod which contains the composition. In general, the processing composition employed in our system contains the developing agent for development, although the composition could also just be an alkaline solution where the developer is incorporated in the photosensitive element, in which case the alkaline solution serves to activate the incorporated developer.

A photographic film unit according to our invention which is adapted to be processed by passing the unit between a pair of juxtaposed pressure-applying members, comprises:

1. a photosensitive element as described above;
2. a dye image-receiving layer; and
3. means for discharging an alkaline processing composition within the film unit such as a rupturable container which is adapted to be positioned during processing of the film unit so that a compressive force applied to the container by the pressure-applying members will effect a discharge of the contents of the container within the film unit; the film unit containing a silver halide developing agent.

The dye image-receiving layer in the above-described film unit can be located on a separate support adapted to be superposed on the photosensitive element after exposure thereof. Such image-receiving elements are generally disclosed, for example, in U.S. Pat. No. 3,362,819. When the means for discharging the processing composition is a rupturable container, typically it is positioned in relation to the photosensitive element and the image-receiving element so that a compressive force applied to the container by pressure-applying members, such as found in a camera designed for in-camera processing, will effect a discharge of the contents of the container between the image-receiving element and the outermost layer of the photosensitive element. After processing, the dye image-receiving element is separated from the photosensitive element.

The dye image-receiving layer in the above-described film unit can also be located integral with the photosensitive silver halide emulsion layer. One useful format for integral receiver-negative photosensitive elements is disclosed in Belgian Pat. No. 757,960. In such an embodiment, the support for the photosensitive element is transparent and is coated with an image-receiving layer, a substantially opaque light reflective layer, e.g.,  $TiO_2$ , and then the photosensitive layer of layers described above. After exposure of the photosensitive element, a rupturable container containing an alkaline processing composition and an opaque process sheet are brought into superposed position. Pressure-applying members in the camera rupture the container and spread processing composition over the photosensitive element as the film unit is withdrawn from the camera. The processing composition develops each exposed silver halide emulsion layer and dye images are formed as a function of development which diffuse to the image-receiving layer to provide a position, right-reading image which is viewed through the transparent support on the opaque reflecting layer background.

Another format for integral negative-receiver photosensitive elements in which the present invention can be employed is disclosed in Belgian Pat. No. 757,959. In this embodiment, the support for the photosensitive element is transparent and is coated with the image-receiving layer, a substantially opaque, light-reflective layer and the photosensitive layer or layers described above. A rupturable container containing an alkaline processing composition and an opacifier is positioned adjacent to the top layer and a transparent top sheet. The film unit is placed in a camera, exposed through the transparent top sheet and then passed through a pair of pressure-applying members in the camera as it is being removed therefrom. The pressure-applying members rupture the container and spread processing com-

position and opacifier over the negative portion of the film unit to render it light insensitive. The processing composition develops each silver halide layer and dye images are formed as a result of development which diffuse to the image-receiving layer to provide a right-reading image that is viewed through the transparent support on the opaque reflecting layer background.

Still other useful integral formats in which our sulfonamido compounds can be employed are described in 10 U.S. Pat. Nos. 3,415,644; 3,415,645; 3,415,646; 3,647,437; and 3,635,707.

The film unit or assembly of the present invention can be used to produce positive images in single or multicolors. In a three-color system, each silver halide 15 emulsion layer of the film assembly will have associated therewith an image dye-providing material possessing a predominant spectral absorption within the region of the visible spectrum to which said silver halide emulsion is sensitive, i.e., the blue-sensitive silver halide 20 emulsion layer will have a yellow image dye-providing material associated therewith, the green-sensitive silver halide emulsion layer will have a magenta image dye-providing material associated therewith, and the red-sensitive silver halide emulsion layer will have a cyan 25 image dye-providing material associated therewith. The image dye-providing material associated with each silver halide emulsion layer can be contained either in the silver halide emulsion layer itself or in a layer contiguous to the silver halide emulsion layer. The cyan 30 image dye-providing material will, of course, be a compound of this invention.

When G is a hydrolyzable acyloxy group, the absorption spectrum of the azo dye is shifted to shorter wavelength. "Shifted dyes" of this type absorb light outside 35 the range to which the associated silver halide layer is sensitive. The use of certain related shifted azo dye developers is described in U.S. Pat. No. 3,307,947 issued Mar. 7, 1967. The shifted dye-providing materials of this invention can be advantageously contained in 40 the silver halide emulsion layer without substantially reducing the sensitivity of the layer. The acyloxy group is hydrolyzed by the alkaline processing composition, releasing the cyan dye of the desired hue. The yellow and magenta image dye-providing materials can be 45 selected from a variety of materials such as those compounds described by Fleckenstein et al U.S. Ser. No. 282,796, mentioned previously. Additional useful magenta image dye-providing materials are described in co-filed Haase et al application Ser. No. 331,729, entitled "Novel Compounds and Photographic Materials."

The concentration of the compounds, which preferably are alkali cleavable upon oxidation, that are employed in the present invention can be varied over a wide range depending upon the particular compound 55 employed and the results which are desired. For example, the image dye-providing compounds of the present invention can be coated in layers as dispersions in a hydrophilic film-forming natural or synthetic polymer, such as gelatin, polyvinyl alcohol, etc., which is 60 adapted to be permeated by aqueous alkaline processing composition. Preferably, the ratio of dye-providing compound to polymer will be about 0.25 to about 4.0. The present compounds may then be incorporated in a gelatin by techniques known in the art (e.g., a high boiling, water immiscible organic solvent or a low boiling or water miscible organic solvent).

Depending upon which Car is used on the present compounds, a variety of silver halide developing agents

can be employed in our invention. If the carrier used is that of Formula III, any silver halide developing agent can be used as long as it cross-oxidizes with the image dye-providing compounds used herein. The developer can be employed in the photosensitive element to be activated by the alkaline processing composition. Specific examples of developers which can be employed in our invention include hydroquinone, aminophenols, e.g., N-methylaminophenol, Phenidone (1-phenyl-3-pyrazolidone) trademark of Ilford, Ltd.; Dimezone (1-phenyl-4,4-dimethyl-3-pyrazolidone) trademark of Eastman Kodak Company; 1-phenyl-4-methyl-4-hydroxymethyl-3-pyrazolidone, N,N-diethyl-p-phenylenediamine, 3-methyl-N,N-diethyl-p-phenylenediamine, 3-methoxy-N,N-diethyl-p-phenylenediamine, etc. The black-and-white developers in this list are preferred, in that they have a reduced propensity of staining the dye image-receiving layer.

In a preferred embodiment of our invention, the silver halide developer in our process becomes oxidized upon development and reduces silver halide to silver metal. The oxidized developer then cross-oxidizes the sulfonamido-phenol or sulfonamido-naphthol dye-releasing compound. The product of cross-oxidation then undergoes alkaline hydrolysis, thus releasing an imagewise distribution of diffusible anionic dye which then diffuses to the receiving layer to provide the dye image. The diffusible moiety is transferable in alkaline processing composition either by virtue of its self-diffusivity or by having attached to it one or more solubilizing groups such as  $-COOH$ ,  $-SO_3H$ ,  $-SO_2NR^5R^6$ , OH, etc. (where  $R^5$  and  $R^6$  are as described previously with at least one being hydrogen).

In using the especially preferred dye-releasing compounds according to our invention, the production of diffusible dye images is a function of development of the silver halide emulsions with a silver halide developing agent to form either negative or direct positive silver images in the emulsion layers. If the silver halide emulsion employed forms a direct positive silver image, such as a direct positive internal-image emulsion or a solarizing emulsion, which develops in unexposed areas, a positive image can be obtained on the dye image-receiving layer. After exposure of the film unit, the alkaline processing composition permeates the various layers to initiate development in the unexposed photosensitive silver halide emulsion layers. The developing agent present in the film unit develops each of the silver halide emulsion layers in the unexposed areas (since the silver halide emulsions are direct-positive ones), thus causing the developing agent to become oxidized imagewise corresponding to the unexposed areas of the direct-positive silver halide emulsion layers. The oxidized developing agent then cross-oxidizes the dye-releasing compounds and the oxidized form of the compounds then undergoes a base-catalyzed reaction in a preferred embodiment of our invention, to release the preformed dyes imagewise as a function of the image-wise exposure of each of the silver halide emulsion layers. At least a portion of the image-wise distributions of diffusible dyes diffuse to the image-receiving layer to form a positive image of the original subject. After being contacted by the alkaline processing composition, a pH-lowering layer in the film unit lowers the pH of the film unit (or the image-receiving unit) to stabilize the image.

Internal-image silver halide emulsions useful in those embodiments wherein a dye is released as a function of

oxidation are direct-positive emulsions that form latent images predominantly inside the silver halide grains, as distinguished from silver halide grains that form latent images predominantly on the surface thereof. Such internal-image emulsions are described by Davey et al in U.S. Pat. No. 2,592,250, issued Apr. 8, 1952, and elsewhere in the literature. Other useful emulsions are described in U.S. Pat. No. 3,761,276, dated Sept. 25, 1973. Internal-image silver halide emulsions can be defined in terms of the increased maximum density obtained when developed with "internal-type" developers over that obtained when developed with "surface-type" developers. Suitable internal-image emulsions are those which, when measured according to normal photographic techniques by coating a test portion of the silver halide emulsion on a transparent support, exposing to a light-intensity scale having a fixed time between 0.01 and 1 second, and developing for 3 minutes at 20°C. in Developer A below ("internal-type" developer), have a maximum density at least five times the maximum density obtained when an equally exposed silver halide emulsion is developed for 4 minutes at 20°C. in Developer B described below ("surface-type" developer). Preferably, the maximum density in Developer A is at least 0.5 density unit greater than the maximum density in Developer B.

| DEVELOPER A                      |       |
|----------------------------------|-------|
| Hydroquinone                     | 15 g. |
| Monomethyl-p-aminophenol sulfate | 15 g. |
| Sodium sulfite (desiccated)      | 50 g. |
| Potassium bromide                | 10 g. |
| Sodium hydroxide                 | 25 g. |
| Sodium thiosulfate               | 20 g. |
| Water to make one liter.         |       |

  

| DEVELOPER B              |        |
|--------------------------|--------|
| P-hydroxyphenylglycine   | 10 g.  |
| Sodium carbonate         | 100 g. |
| Water to make one liter. |        |

The internal-image silver halide emulsions when processed in the presence of fogging or nucleating agents provide direct positive silver images. Such emulsions are particularly useful in the above-described embodiment. Suitable fogging agents include the hydrazines disclosed in Ives U.S. Pat. Nos. 2,588,982 issued Mar. 11, 1952, and 2,563,785 issued Aug. 7, 1951; the hydrazides and hydrazones disclosed in Whitmore U.S. Pat. No. 3,227,552 issued Jan. 4, 1966; hydrazone quaternary salts described in Lincoln and Heseltine U.S. Pat. No. 3,615,615 issued Oct. 16, 1971; hydrazone containing polymethine dyes described in Spence and Janssen U.S. Pat. No. 3,718,470 issued Feb. 27, 1973; or mixtures thereof. The quantity of fogging agent employed can be widely varied depending upon the results desired. Generally, the concentration of fogging agent is from about 0.4 to about 8 grams per mole of silver in the photosensitive layer in the photosensitive element or from about 0.1 to about 2 grams per liter of developer if it is located in the developer. The fogging agents described in U.S. Pat. Nos. 3,615,615 and 3,718,470, however, are preferably used in concentrations of about 0.5 to 10.0 grams per mole of silver in the photosensitive layer.

The solarizing direct-positive silver halide emulsions useful in the above-described embodiment are well-known silver halide emulsions which have been effectively fogged either chemically, such as by the use of

reducing agents, or by radiation to a point which corresponds approximately to the maximum density of the reversal curve as shown by Mees, *The Theory of the Photographic Process*, published by the Macmillan Co., New York, New York, 1942, pages 261-297. Typical methods for the preparation of solarizing emulsions are shown by Groves British Pat. No. 443,245, Feb. 25, 1936, who subjected emulsions to Roentgen rays "until an emulsion layer formed therefrom, when developed without preliminary exposure, is blackened up to the apex of its graduation curve"; Szaz British Pat. No. 462,730, Mar. 15, 1937, the use of either light or chemicals such as silver nitrate, to convert ordinary silver halide emulsions to solarizing direct positive emulsions; and Arens U.S. Pat. No. 2,005,837, June 25, 1935, the use of silver nitrate and other compounds in conjunction with heat to effect solarization. Particularly useful are the fogged direct-positive emulsions of Berriman U.S. Pat. No. 3,367,778; Illingsworth U.S. Pat. Nos. 3,501,305, 3,501,306 and 3,501,307; and combinations thereof.

Other embodiments in which our imaging chemistry can be employed include the techniques described in U.S. Pat. Nos. 3,227,550, 3,227,551, 3,227,552 and 3,364,022.

If photographic elements are used which contain compounds of this invention wherein Car is a silver halide developer as described, for example, in U.S. Pat. No. 2,983,606, when the liquid processing composition is applied, it permeates the emulsion to provide a solution of the dye developer substantially uniformly distributed in the emulsion. As the exposed silver halide emulsion is developed to a negative silver image, the oxidation product of the dye developer is immobilized or precipitated in situ with the developed silver, thereby providing an imagewise distribution of unoxidized dye developer dissolved in the liquid processing composition. This immobilization is apparently due, at least in part, to a change in the solubility characteristics of the dye developer upon oxidation. At least part of this imagewise distribution of unoxidized dye-developer is transferred to a superposed image-receiving layer to provide a transfer image.

Negative silver halide emulsions useful in certain embodiments of this invention, such as the above, can comprise, for example, silver chloride, silver bromide, silver chlorobromide, silver bromoiodide, silver chlorobromoiodide or mixtures thereof. The emulsions can be coarse-or fine-grain and can be prepared by any of the well-known procedures, e.g., single-jet emulsions such as those described in Trivelli and Smith, *The Photographic Journal*, Vol. LXXIX, May, 1939 (pp. 330-338), double-jet emulsions, such as Lippmann emulsions, ammoniacal emulsions, thiocyanate or thioether ripened emulsions such as those described in Nietz et al U.S. Pat. No. 2,222,264 issued Nov. 19, 1940; Illingsworth U.S. Pat. No. 3,320,069 issued May 16, 1967; and Jones U.S. Pat. No. 3,574,628 issued Apr. 13, 1971. The emulsions may be monodispersed regular-grain emulsions such as the type described in Klein and Moisar, *J. Phot. Sci.*, Vol. 12, No. 5, Sept./Oct., 1964 (pp. 242-251).

Another embodiment of our invention uses the image-reversing technique disclosed in British Pat. No. 904,364, page 19, lines 1-41. In this system our dye-providing compounds are used in combination with physical development nuclei in a nuclei layer contiguous to the photosensitive silver halide negative emul-

sion layer. The film unit contains a silver halide solvent, preferably in a rupturable container with the alkaline processing composition.

The various silver halide emulsion layers of a color film assembly of the invention can be disposed in the usual order, i.e., the blue-sensitive silver halide emulsion layer first with respect to the exposure side, followed by the green-sensitive and red-sensitive silver halide emulsion layers. If desired, a yellow dye layer or a yellow colloidal silver layer can be present between the blue-sensitive and green-sensitive silver halide emulsion layer for absorbing or filtering blue radiation that may be transmitted through the blue-sensitive layer. If desired, the selectivity sensitized silver halide emulsion layers can be disposed in a different order, e.g., the blue-sensitive layer first with respect to the exposure side, followed by the red-sensitive and green-sensitive layers.

The rupturable container employed in this invention can be of the type disclosed in U.S. Pat. Nos. 2,543,181; 2,643,886; 2,653,732; 2,724,051; 3,056,492; 3,056,491 and 3,152,515. In general, such containers comprise a rectangular sheet of fluid- and air-impervious material folded longitudinally upon itself to form two walls which are sealed to one another along their longitudinal and end margins to form a cavity in which processing solution is contained.

In a color film unit according to this invention, each silver halide emulsion layer containing a dye image-providing material or having the dye image-providing material present in a contiguous layer may be separated from the other silver halide emulsion layers in the image-forming portion of the film unit by materials including gelatin, calcium alginate, or any of those disclosed in U.S. Pat. No. 3,384,483, polymeric materials such as polyvinylamides as disclosed in U.S. Pat. No. 3,421,892, or any of those disclosed in French Pat. No. 2,028,236 or U.S. Pat. Nos. 2,992,104; 3,043,692; 3,044,873; 3,061,428; 3,069,263; 3,069,264; 3,121,011; and 3,427,158.

Generally speaking, except where noted otherwise, the silver halide emulsion layers in the invention comprise photosensitive silver halide dispersed in gelatin and are about 0.6 to 6 microns in thickness; the dye image-providing materials are dispersed in an aqueous alkaline solution-permeable polymeric binder, such as gelatin, as a separate layer about 1 to 7 microns in thickness; and the alkaline solution-permeable polymeric interlayers, e.g., gelatin, are about 1 to 5 microns in thickness. Of course, these thicknesses are approximate only and can be modified according to the product desired.

Any material can be employed as the image-receiving layer in this invention as long as the desired function of mordanting or otherwise fixing the dye images will be obtained. The particular material chosen will, of course, depend upon the dye to be mordanted. If acid dyes are to be mordanted, the image-receiving layer can contain basic polymeric mordants such as polymers of amino guanidine derivatives of vinyl methyl ketone such as described in Minsk U.S. Pat. No. 2,882,156, issued Apr. 14, 1959, and basic polymeric mordants such as described in Cohen et al U.S. Pat. No. 3,625,694, issued Dec. 7, 1971; U.S. Pat. No. 3,709,690, issued Jan. 9, 1973; and U.S. application Ser. No. 400,778, filed Sept. 26, 1973. See also U.S. application Ser. No. 412,992 of Burness et al, filed Nov. 5, 1973.

Preferred mordants are cationic mordants such as polymeric compounds composed of a polymer having quaternary nitrogen groups and at least two aromatic nuclei for each quaternary nitrogen in the polymer cation (i.e., having at least two aromatic nuclei for each positively charged nitrogen atom), such polymeric compounds being substantially free of carboxy groups. Useful mordants of this type are comprised of units of the following formula in copolymerized relationship with units of at least one other ethylenically unsaturated monomer:



wherein R<sup>7</sup> and R<sup>8</sup> each represent a hydrogen atom or a lower alkyl radical (of 1 to about 6 carbon atoms) and R<sup>8</sup> can additionally be a group containing at least one aromatic nucleus (e.g., phenyl, naphthyl, tolyl); Q can be a divalent alkylene radical (of 1 to about 6 carbon atoms), a divalent arylene radical, a divalent aralkylene radical, a divalent arylenealkylene radical, such as



wherein R<sup>12</sup> is an alkylene radical, or R<sup>8</sup> can be taken together with Q to form a



group; R<sup>8</sup>, R<sup>10</sup> and R<sup>11</sup> can be alkyl, aralkyl or aryl, or R<sup>8</sup> and R<sup>10</sup> and the nitrogen atom to which they are attached can together with Q represent the atoms and bonds necessary to form a quaternized nitrogen-containing heterocyclic ring, and X<sup>-</sup> is a monovalent negative salt-forming radical or atom in ionic relationship with the positive salt-forming radical, wherein said polymer is substantially free of carboxy groups and wherein the positive salt-forming radical of said polymer comprises at least two aryl groups for each quaternary nitrogen atom in said polymer. In one preferred embodiment, Q represents a phenylene or substituted phenylene radical and R<sup>8</sup>, R<sup>10</sup> and R<sup>11</sup> are the same or different and represent alkyl groups, the sum of their carbon atoms exceeding 12. These preferred polymeric cationic mordants are described further in the above-mentioned U.S. Pat. No. 3,709,690 and U.S. application Ser. No. 400,778, incorporated herein by reference.

Other mordants useful in our invention include poly-4-vinylpyridine, the 2-vinyl pyridine polymer methyl-p-

toluene sulfonate and similar compounds described in Sprague et al U.S. Pat. No. 2,484,430, issued Oct. 11, 1949, and cetyl trimethylammonium bromide, etc. Effective mordanting compositions are also described in Whitmore U.S. Pat. No. 3,271,148 and Bush U.S. Pat. No. 3,271,147, both issued Sept. 6, 1966.

Generally, good results are obtained when the image-receiving layer, preferably alkaline solution-permeable, is transparent and about 0.25 to about 0.40 mil in thickness. This thickness, of course, can be modified depending upon the result desired. The image-receiving layer can also contain ultraviolet absorbing materials to protect the mordanted dye images from fading due to ultraviolet light, brightening agents such as the stilbenes, coumarins, triazines, oxazoles, dye stabilizers such as the chromanols, alkylphenols, etc.

Use of a pH-lowering material in the dye image-receiving element of a film unit according to the invention will usually increase the stability of the transferred image. Generally, the pH-lowering material will effect a reduction in the pH of the image layer from about 13 or 14 to at least 11 and preferably 4-8 within a short time after imbibition. For example, polymeric acids as disclosed in U.S. Pat. No. 3,362,819, or solid acids or metallic salts, e.g., zinc acetate, zinc sulfate, magnesium acetate, etc., as disclosed in U.S. Pat. No. 2,584,030 may be employed with good results. Such pH-lowering materials reduce the pH of the film unit after development to terminate development and substantially reduce further dye transfer and thus stabilize the dye image.

An inert timing or spacer layer can be employed in the practice of our invention over the pH-lowering layer which "times" or controls the pH reduction as a function of the rate at which alkali diffuses through the inert spacer layer. Examples of such timing layers include gelatin, polyvinyl alcohol or any of those disclosed in U.S. Pat. No. 3,455,686. The timing layer may be effective in evening out the various reaction rates over a wide range of temperatures, e.g., premature pH reduction is prevented when imbibition is effected at temperatures above room temperature, for example, at 95°-100°F. The timing layer is usually about 0.1 to about 0.7 mil in thickness. Especially good results are obtained when the timing layer comprises a hydrolyzable polymer or a mixture of such polymers which are slowly hydrolyzed by the processing composition. Examples of such hydrolyzable polymers include polyvinyl acetate, polyamides, cellulose esters, etc.

The alkaline processing composition employed in this invention is the conventional aqueous solution of an alkaline material, e.g., sodium hydroxide, sodium carbonate or an amine such as diethylamine, preferably possessing a pH in excess of 11, and preferably containing a developing agent as described previously. The solution also preferably contains a viscosity-increasing compound such as a high-molecular-weight polymer, e.g., a water-soluble ether inert to alkaline solutions such as hydroxyethyl cellulose or alkali metal salts of carboxymethyl cellulose such as sodium carboxymethyl cellulose. A concentration of viscosity-increasing compound of about 1 to about 5 percent by weight of the processing composition is preferred which will impart thereto a viscosity of about 100 cp. to about 200,000 cp. In certain embodiments of our invention, an opacifying agent, e.g., TiO<sub>2</sub>, carbon black, pH indicator dyes, etc., may be added to the processing composition.

While the alkaline processing composition used in this invention can be employed in a rupturable container, as described previously, to conveniently facilitate the introduction of processing composition into the film unit, other methods of inserting processing composition into the film unit could also be employed, e.g., interjecting processing solution with communicating members similar to hypodermic syringes which are attached either to a camera or camera cartridge.

The alkaline solution-permeable, substantially opaque, light-reflective layer employed in certain embodiments of photographic film units of our invention can generally comprise any opacifier dispersed in a binder as long as it has the desired properties. Particularly desirable are white light-reflective layers since they would be esthetically pleasing backgrounds on which to view a transferred dye image and would also possess the optical properties desired for reflection of incident radiation. Suitable opacifying agents include titanium dioxide, barium sulfate, zinc oxide, barium stearate, silver flake, silicates, alumina, zirconium oxide, zirconium acetyl acetate, sodium zirconium sulfate, kaolin, mica, or mixtures thereof in widely varying amounts depending upon the degree of opacity desired. The opacifying agents may be dispersed in any binder such as an alkaline solution-permeable polymeric matrix such as, for example, gelatin, polyvinyl alcohol, and the like. Brightening agents such as the stilbenes, coumarins, triazines and oxazoles can also be added to the light-reflective layer, if desired. When it is desired to increase the opacifying capacity of the light-reflective layer, dark-colored opacifying agents, e.g., carbon black, nigrosine dyes, etc., may be added to it, or coated in a separate layer adjacent to the light-reflective layer.

The supports for the photographic elements of this invention can be any material as long as it does not deleteriously effect the photographic properties of the film unit and is dimensionally stable. Typical flexible sheet materials include cellulose nitrate film, cellulose acetate film, poly(vinyl acetal) film, polystyrene film, poly(ethyleneterephthalate) film, polycarbonate film, poly- $\alpha$ -olefins such as polyethylene and polypropylene film, and related films or resinous materials. The support can be from about 2 to about 9 mils in thickness.

The silver halide emulsions useful in our invention are well known to those skilled in the art and are described in *Product Licensing Index*, Vol. 92, December, 1971, publication 9232, p. 107, paragraph I, "Emulsion types"; they may be chemically and spectrally sensitized as described on page 107, paragraph III, "Chemical sensitization," and pp. 108-109, paragraph XV, "Spectral sensitization," of the above article; they can be protected against the production of fog and can be stabilized against loss of sensitivity during keeping by employing the materials described on p. 107, paragraph V, "Antifoggants and stabilizers," of the above article; they can contain development modifiers, hardeners, and coating aids as described on pp. 107-108, paragraph IV, "Development modifiers"; paragraph VII, "Hardeners"; and paragraph XII, "Coating aids", of the above article; they and other layers in the photographic elements used in this invention can contain plasticizers, vehicles and filter dyes described on p. 108, paragraph XI, "Plasticizers and lubricants," and paragraph VIII, "Vehicles," and p. 109, paragraph XVI, "Absorbing and filter dyes," of the above article; they and other layers in the photographic elements

used in this invention may contain addenda which are incorporated by using the procedures described on p. 109, paragraph XVII, "Methods of addition," of the above article; and they can be coated by using the various techniques described on p. 109, paragraph XVIII, "Coating procedures," of the above article, the disclosures of which are hereby incorporated by reference.

It will be appreciated that there remains in the photographic element after transfer has taken place an imagewise distribution of dye in addition to developed silver. A color image comprising residual nondiffusible compound may be obtained in this element if the residual silver and silver halide are removed by any conventional manner well known to those skilled in the photographic art, such as a bleach bath followed by a fix bath, a bleach-fix bath, etc. The imagewise distribution of dye may also diffuse out of the element into these baths, if desired, rather than to an image-receiving element. If a negative-working silver halide emulsion is employed in such photosensitive element, then a positive color image, such as a color transparency or motion-picture film, may be produced in this manner. If a direct-positive silver halide emulsion is employed in such photosensitive element, then a negative color image may be produced.

Preferably, when the desired dye image is retained in the image-forming unit, the image dye-providing materials are shifted (G is hydrolyzable acyloxy) and are incorporated in the silver halide emulsion layer. Improved processes are described in U.S. Ser. No. 422,390, filed Dec. 6, 1973.

The following examples are provided for a further understanding of the invention. The structures of all of the compounds were confirmed by their infrared and NMR spectra and in some cases by elemental analysis. The notation  $C_5H_{11}-t$  as used herein as an abbreviation for t-pentyl.

#### EXAMPLE 1 - PREPARATION OF COMPOUND No. 1



A mixture of 3.05 g. (0.0065 mol) of 5-hydroxy-8-(2-methylsulfonyl-4-nitrophenylazo)-2-naphthalenesulfonyl chloride and 3.2 g. (0.0065 mol) of 4-amino-N-[4-(2,4-di-t-pentylphenoxy)-butyl]-1-hydroxy-2-naphthamide in 75 ml. of tetrahydrofuran under nitrogen was stirred with 4.5 ml. of pyridine at room temperature for ninety minutes. The solid, precipitated by dilution with 500 ml. with hexane, was collected on a filter funnel and dried to yield 4.8 g. (80 percent). The solid was purified by dissolving the soluble material in tetrahydrofuran and reprecipitating with hexane. The still slightly impure solid was chromatographed on silica

gel, the product being eluted with tetrahydrofuran. The eluents were concentrated and the solid precipitated with hexane. The yield was 2.2 g. (37 percent), m.p. 170°-3°C.

#### PREPARATION OF INTERMEDIATES

a. The 5-hydroxy-8-(2-methylsulfonyl-4-nitrophenylazo)-2-naphthalenesulfonyl chloride was prepared from the sodium salt of the acid with chlorosulfonic acid; 3.55 g. (0.0075 mol) of sodium 5-hydroxy-8-(2-methylsulfonyl-4-nitrophenylazo)-2-naphthalenesulfonate in 35 ml. of chlorosulfonic acid was heated at 60°C. for one hour. The solution was cooled and poured onto ice. The solid was collected on a filter funnel and dried in a vacuum desiccator to yield 2.8 g. (80 percent) of the product which contained a small amount of starting material.

b. The sodium 5-hydroxy-8-(2-methylsulfonyl-4-nitrophenylazo)-2-naphthalenesulfonate was prepared by the following diazotization and coupling reactions. To a solution of 55.8 g. (0.25 mol) of 1-amino-6-naphthalenesulfonic acid in 100 ml. of water containing 10 g. (0.25 mol) of sodium hydroxide was added 17.3 g. (0.25 mol) of sodium nitrite in 50 ml. of water. At 0°-5°C., a dilute solution of sulfuric acid, formed by adding 50 g. of ice to 125 ml. of concentrated sulfuric acid was added dropwise. After one hour, the solution was poured into a 3 liter flask and slowly heated to reflux (gas evolved at 70°-90°C.). The solution was heated at reflux for 1½ hours, cooled, pH adjusted to 7 using 50 percent sodium hydroxide, and an additional 425 g. of 50 percent sodium hydroxide was added (Solution A). 17.3 g. (0.25 mol) of sodium nitrite was added portionwise to 150 ml. of concentrated sulfuric acid at 0°C. The mixture was allowed to warm to 70°C., cooled to 10°C., and 54 g. (0.25 mol) of 2-amino-5-nitrophenyl methyl sulfone was added. The mixture was stirred for ninety minutes and poured onto 625 g. of ice. The mixture was filtered and the filtrates kept (Solution B). Solution B was added to Solution A at <30°C. After the addition, the pH was adjusted to 5 and the mixture stirred for one-half hour. The solid was collected on a filter funnel, reslurried in water. After collecting the solid on a filter funnel and drying, the yield of product was 85 g. (72%).

#### EXAMPLE 2 - Preparation of Compound No. 2



To a mixture of 4.2 g. (0.009 mol) of 5-hydroxy-8-(2-methylsulfonyl-4-nitrophenylazo)-1-naphthalenesulfonyl chloride and 4.4 g. (0.009 mol) of 4-amino-N-[4-(2,4-di-t-pentylphenoxy)-butyl]-1-hydroxy-2-naphthamide in 100 ml. of tetrahydrofuran under nitrogen, was added 4.5 ml. of pyridine. The solution was stirred at room temperature for two hours, and diluted to 800 ml. with hexane. The solid was collected on a filter funnel and dried to yield 4.8 g. (58 percent) of crude product.

The solid was chromatographed on a silica column, using tetrahydrofuran to elute the desired product. Concentration of the eluents yielded 3.2 g. of slightly impure solid. After twice suspending the solid in 200 ml. of chloroform and diluting with 400 ml. of hexane, the yield of purified product was 2.4 g. (29 percent), m.p. 195°-6°C. dec.

#### PREPARATION OF INTERMEDIATES

a. The 5-hydroxy-8-(2-methylsulfonyl-4-nitrophenylazo)-1-naphthalenesulfonyl chloride was prepared from the corresponding sodium sulfonate. 23.9 g. (0.05 mol) of sodium 5-hydroxy-8-(2-methylsulfonyl-4-nitrophenylazo)-1-naphthalenesulfonate in 150 ml. of chlorosulfonic acid was heated at 65°C. for one hour. The mixture was cooled and poured onto ice. The mixture was kept at <5°C. by addition of ice until filtration was complete. The solid was collected on a filter funnel and dried in a vacuum desiccator to yield 18.4 g. (78 percent). The solid was dissolved in 150 ml. of tetrahydrofuran and diluted with 600 ml. of chloroform. The solid that precipitated was collected on a filter funnel and discarded. The filtrates were chromatographed on a silica column, which chloroform being used to elute the product. The chloroform eluents were concentrated to dryness to yield 5.4 g. (23 percent) of purified product.

b. The sodium 5-hydroxy-8-(2-methylsulfonyl-4-nitrophenylazo)-1-naphthalenesulfonate was prepared using the method shown in Example 1 by substituting a solution of 1-naphthol-5-sulfonic acid in dilute sodium hydroxide for solution A. The yield was 100 percent.

c. 4-amino-N-[4-(2,4-di-t-pentylphenoxy)-butyl]-1-hydroxy-2-naphthamide may be prepared as follows: 1-hydroxy-N-[4-(2,4-di-t-pentylphenoxy)-butyl]-2-naphthamide (U.S. Patent 2,474,293) is coupled with a diazotized p-anisidine (eg.



The azo group of the compound thus prepared may then be reduced with sodium dithionite (Na2S2O4) to the corresponding amine.

#### EXAMPLE 3 - Preparation of Compound No. 3



This compound was prepared in a manner similar to Example 1. After one recrystallization from ethyl acetate, the yield was 46 percent, m.p. 162°-4°C. dec.

#### PREPARATION OF INTERMEDIATES

a. 5-Hydroxy-8-(2-chloro-4,6-dinitrophenylazo)-2-naphthalenesulfonyl chloride: 9.5 g. (0.02 mol) of so-

25

dium 5-hydroxy-8-(2-chloro-4,6-dinitrophenylazo)-2-naphthalenesulfonate was added portionwise to 20 ml. of chlorosulfonic acid. 20 ml. of thionyl chloride was added and the mixture heated at 60°C. for thirty minutes. The solution was cooled, poured onto ice, and filtered. The wet solid was dissolved in 800 ml. of  $\text{CHCl}_3$  and dried with magnesium sulfate. The mixture was filtered to remove the magnesium sulfate, filtrates concentrated to dryness. The resulting solid was slurried in hexane, collected on a filter funnel and dried to yield 6.7 g. (71 percent). No impurities could be detected by thin-layer chromatography.

b. Sodium 5-hydroxy-8-(2-chloro-4,6-dinitrophenylazo)-2-naphthalenesulfonate: 55.8 g. (0.25 mol) of 1-amino-6-naphthalenesulfonic acid was dissolved in 100 ml. of water containing 10 g. (0.25 mol) of sodium hydroxide. To this solution was added 17.3 g. (0.25 mol) of sodium nitrite in 50 ml. of water. At 0 to 5°C. this was added drop-wise to a dilute solution of sulfuric acid, formed by adding 50 g. of ice to 125 ml. of concentrated sulfuric acid. After 1 hour, the solution was poured into a 3 liter flask and slowly heated to reflux (gas evolved at 70°-90°C.). The solution was heated at reflux for 1½ hours, cooled (Solution A). To 125 ml. of a mixture of 2 parts propionic to 5 parts acetic acids containing 25 drops of Triton X-100 (trademark of Rohm & Haas Company for a nonionic isoctyl phenol polyethoxy ethanol dispersing agent) was added 66 g. of 82 percent solid 2-chloro-4,6-dinitroaniline as a fine powder. The mixture was stirred for 1½ hours at room temperature then at 40°C. for one hour. The mixture was cooled to 0°C. and to it was added slowly at 10°C. a solution formed by adding 17.3 g. (0.25 mol) of sodium nitrite to a concentrated sulfuric acid at 10°C., warming to 70°C. to effect solution, and cooling to 20°C. After the addition, 125 ml. of the propionic-acetic acid mixture in 50 g. of ice was added. The solution was stirred for 2 hours at 10°-15°C., urea added to scavenge excess nitrite. After stirring for thirty minutes, the mixture was filtered to remove starting material and the filtrates taken as Solution B. Solution B was added dropwise to Solution A at -10° to -5°C. The mixture was stirred for thirty minutes, solid collected on a filter funnel and dried to yield 148 g. (125 percent) of material containing salts which are readily removed in subsequent steps.

#### EXAMPLE 4 - Preparation of Compound No. 4



The method used in Example 1 was used to prepare this compound from the following sulfonyl chloride. The yield was 6 percent, m.p. 241°-2°C. dec. The 4-acetamido-5-hydroxy-8-(2-methylsulfonyl-4-nitrophenylazo)-1-naphthalenesulfonic acid used was prepared by the method shown in Example 3 from the following sulfonic acid. The yield was 50 percent. The 4-acetamido-5-hydroxy-8-(2-methylsulfonyl-4-nitrophenylazo)-1-naphthalenesulfonic acid used was pre-

26

pared in a manner similar to Example 1 using a solution of 4-acetamido-5-hydroxy-1-naphthalenesulfonic acid in dilute sodium hydroxide in place of Solution A. The yield was 75 percent.

#### EXAMPLE 5 - Preparation of Compound No. 5



10 This compound was prepared in a manner similar to that used in Example 1. The yield was 23 percent, m.p. 153°-6°C. dec. The 5-hydroxy-8-(4-nitro-2-trifluoromethylphenylazo)-2-naphthalenesulfonyl chloride for use in this reaction was prepared using the method explained in Example 1. The yield was 70%. The sodium 5-hydroxy-8-(4-nitro-2-trifluoromethylphenylazo)-2-naphthalenesulfonate was prepared in a manner similar to that used in Example 1. The apparent yield was 107 percent, due to the presence of salt. It was used without purification in the preparation of the acid chloride.

#### EXAMPLE 6 - Preparation of Compound No. 6



35 The method used in Example 1 was used to prepare this compound. The yield was 19 percent, m.p. 268°-70°C. dec. The 4-acetamido-5-hydroxy-8-(2-

methylsulfonyl-4-nitrophenylazo)-2-naphthalenesulfonyl chloride was prepared in a manner similar to that used for Example 3. The yield was 69 percent. The 4-acetamido-5-hydroxy-8-(2-methylsulfonyl-4-nitrophenylazo)-2-naphthalenesulfonic acid was prepared by a similar method to that used in Example 1 using a basic solution of 4-acetamido-5-hydroxy-2-naphthalenesulfonic acid in place of Solution A. The yield was 100 percent.

## EXAMPLE 7 - Preparation of Compound No. 7



This compound was prepared in a manner similar to that used in Example 1. The yield was 16 percent, m.p. 248°-9°C. dec. The 4-butyramido-5-hydroxy-8-(2-methylsulfonyl-4-nitrophenylazo)-2-naphthalenesulfonyl chloride was prepared by the method explained in Example 3. The yield was 86 percent. The 4-butyramido-5-hydroxy-8-(2-methylsulfonyl-4-nitrophenylazo)-2-naphthalenesulfonic acid was prepared by a method similar to that used in Example 6.

## EXAMPLE 8 - Preparation of Compound No. 8



To a mixture of 3.2 g. (0.006 mol) of 4-acetamido-5-hydroxy-8-(2-methylsulfonyl-4-nitrophenylazo)-2-naphthalenesulfonyl chloride and 3.9 g. (0.006 mol) of 4-(m-aminobenzenesulfonamido)-N-[4-(2,4-di-tert-pentylphenoxy)butyl]-1-hydroxy-2-naphthamide in 75 ml.

45

This compound was prepared in a manner similar to that used in Example 8 in 16 percent yield, m.p. indistinct.

## EXAMPLE 9 - Preparation of Compound No. 9

## 5 EXAMPLE 9 - Preparation of Compound No. 9



of tetrahydrofuran was added 3.0 ml. of pyridine. The mixture was stirred at room temperature for one hour, under nitrogen, then filtered and the filtrates diluted to 500 ml. with hexane. The solid was collected on a filter

This compound was prepared in a manner similar to that used in Example 8 except that it was chromatographed in the presence of diisopropylethylamine. The yield was 17 percent, m.p. <150°C.

funnel and dried. After chromatography of the solid using silica gel and ethyl acetate, the yield of product was 1.0 g. (15 percent) with indistinct m.p.

## EXAMPLE 11 - Preparation of Compound No. 11



This compound was prepared via the method explained in Example 1, in 50 percent yield, m.p. 195°-7°C. dec. The 4-acetamido-8-(2-chloro-4,6-dinitrophenylazo)-5-hydroxy-2-naphthalenesulfonic chloride was prepared in a manner similar to Example 3 in 85 percent yield. The 4-acetamido-8-(2-chloro-4,6-dinitrophenylazo)-5-hydroxy-2-naphthalenesulfonic acid was prepared via the method used in Example 3 in 53 percent yield.

## EXAMPLE 12 - Photographic Testing

The above image dye-providing compounds were tested for reactivity and diffusibility of their released dyes to a receiving element. Each compound was dissolved in an equal weight of diethylauramide and finely dispersed in gelatin. The dispersion was added to a 0.8  $\mu\text{m}$  monodispersed negative-working gelatino-silver bromide emulsion which was coated on a polyester film support, the coverage of compound being about  $1.1 \times 10^{-5}$  moles/dm $^2$ ; silver - 9.2 mg/dm $^2$ ; and gelatin - 32 mg/dm $^2$ . An overcoat layer of 8.6 g/dm $^2$  of gelatin, hardened by formaldehyde was then applied.

A. Image discrimination - A sample of the above coating was exposed through a step-wedge and then laminated to a mordant-containing receiving element with a viscous processing composition (goo) by passing

no transfer of dye in the unexposed areas. The Dmax and Dmin for each transfer is given under image discrimination in the table.

B. Spectrophotometry - The spectra of the released dyes when adsorbed to the mordant on a transparent support were measured spectrophotometrically. The maximum wavelength ( $\lambda_{\text{max}}$ ) and the bandwidth in nm at one-half the density at the  $\lambda_{\text{max}}$  of the curve for each dye is also given in the table. This "half bandwidth" along with the  $\lambda_{\text{max}}$  is indicative of hue, the brightness and purity of color being greater, the smaller the half bandwidth.

C. Dye-transfer in receiving element - Another sample of an emulsion coating containing the image dye-providing compound was fogged by exposure to light and processed by passing it has a "sandwich" with an image receiving element and viscous developing composition (goo) between a pair of juxtaposed pressure-applying rollers. The developer layer thickness of the resulting laminate ranged from about 0.075 to 0.10 mm. The receiving element had the following structure (the coverages in mg/dm $^2$  are shown in parenthesis):

25 Carbon (27) + Gelatin (17)

TiO<sub>2</sub> (215) + Gelatin (21)

Mordant\* (21) + Gelatin (11)

Cellulose acetate support

\*Same as above.

The "goo" contained 20 g. sodium hydroxide, 0.75 g. 30 4-hydroxymethyl-4-methyl-1-phenyl-3-pyrazolidone, 10 g. potassium bromide and 25 g. hydroxyethylcellulose, all per liter of solution. Upon application of the goo to the fogged emulsion layer, the dyes are released and diffuse through the carbon and titania layers to the mordant layer. The density of the dyes on the mordant layer was read through the support by means of a reflection densitometer after intervals of 30, 60 and 120 seconds at 24°C. The increase in density, as indicated by the values in the table, is a measure of the rate of release and also of the diffusivity of the dyes.

35

40

| Compound of Example | max (nm) | width (nm) | PHOTOGRAPHIC PROPERTIES                           |      |      |                                       | Density of Dye Transfer Image |         |          |
|---------------------|----------|------------|---------------------------------------------------|------|------|---------------------------------------|-------------------------------|---------|----------|
|                     |          |            | Image Discrimination                              |      |      | Coverage                              |                               |         |          |
|                     |          |            | Coverage<br>(moles $\times 10^{-6}$ per dm $^2$ ) | Dmax | Dmin | (moles $\times 10^{-6}$ per dm $^2$ ) | 30 sec.                       | 60 sec. | 120 sec. |
| 1                   | 639      | 119        | 11                                                | 2.70 | 0.72 | 11                                    | 0.33                          | 0.84    | 2.04     |
| 2                   | 634      | 113        | 11                                                | 1.80 | 0.70 | 11                                    | 0.35                          | 1.04    | 1.92     |
| 3                   | 645      | 115        | 11                                                | 2.60 | 0.44 | 11                                    | 0.64                          | 1.48    | 2.30     |
| 4                   | 645      | 133        | 11                                                | 3.20 | 1.46 | 11                                    | 0.77                          | 1.29    | 1.78     |
| 5                   | 637      | 132        | 11                                                | 1.20 | 0.20 | 6                                     | 0.24                          | 0.35    | 0.58     |
| 6                   | 615      | 130        | 6                                                 | 1.52 | 0.50 | 6                                     | 0.36                          | 0.71    | 1.10     |
| 7                   | 622      | 132        | 6                                                 | 2.10 | 0.71 | 6                                     | 0.32                          | 0.76    | 1.43     |
| 8                   | 669      | 114        | 6                                                 | 3.00 | 0.52 | 6                                     | 0.51                          | 1.11    | 1.98     |
| 9                   | 653      | 110        | 6                                                 | 1.45 | 0.50 | 6                                     | 0.42                          | 0.89    | 1.50     |
| 10                  | 640      | 122        | 6                                                 | 2.70 | 0.68 | 6                                     | 0.81                          | 1.63    | 2.35     |
| 11                  | 660      | 120        | 11                                                | 2.84 | 0.56 | 6                                     | 0.20                          | 0.46    | 0.85     |

the "sandwich" between a pair of juxtaposed pressure-applying rollers. The receiving element consisted of a paper support on which was coated a mixture of gelatin (21 mg/dm $^2$ ) and a mordant, poly[styrene-co-N-benzyl-N,N-dimethyl-N-(3-maleimidopropyl)ammonium chloride] (21 mg/dm $^2$ ). The goo contained, per liter of solution, 20 g. sodium hydroxide, 0.75 g. 4-hydroxymethyl-4-methyl-1-phenyl-3-pyrazolidone, 10 g. potassium bromide and 25 g. hydroxyethylcellulose. After 60 seconds, the receiver was peeled apart and washed in water to adjust the pH to about 7. Good image density in the exposed areas was obtained with practically

## EXAMPLE 13 - Preparation of Compounds 12 and 12a

60 A mixture of 3 g. NaHCO<sub>3</sub>, 4.93 g. (8.10 mmol) Compound A, and 3.97 g. (8.10 mmol) of 1-hydroxy-4-amino-N-[4-(2,4-di-t-pentylphenoxy)-butyl]-2-naphthamide (referred to below as NH<sub>2</sub>- Group) in 30 g. dry dimethylsulfoxide was stirred at 80°-100°C. for 60 minutes, cooled and poured onto ice water containing sufficient dilute HCl to neutralize the excess NaHCO<sub>3</sub>. The precipitated Compound 12 was filtered, washed with water, and air dried (crude dye cake yield = 102 percent). Compound 12 was quite clean as isolated but

was chromatographed on a silica gelcellulose (equal parts by weight) dry packed column by ascending development with a solution of ethyl acetate (9 parts by volume) and methanol (1 part by volume). A schematic representation of the reactions involved is shown below:

cooled to 5°C. Meanwhile, a solution of 1.2 g. 2-amino-5-nitrobenzenesulfonic acid sodium salt (5.00 mmol) and 0.036 g. sodium nitrite (5.00 mmol) in 50 ml. water was cooled to 0°C. and added dropwise to a solution of 1 ml. 37 percent HCl in 20 ml. of water at 0°C. The diazotization was very rapid--the resulting

Step 1Step 2

A.

Step 3

The compound was tested as in Example 12 and the released dye had a  $\lambda_{max}$  of 640 nm and Dmax of 2.35 at 60 seconds and 2.5 at 120 seconds. A similar compound (Compound 12a) having a cyano radical in place of the methylsulfonyl on the nitrophenyl ring also gave good results.

## EXAMPLE 14 - Preparation of Compounds 13, 13a, 13b and 13c

A solution of 4.14 (5.00 mmol) of Coupler A in 20 ml. pyridine and 150 ml. 1:5 acid [propionic acid (1 volume):acetic acid (5 volumes)] was prepared and

suspension of diazonium salt was slowly added at 5°C. to the coupler solution. The coupling was rapid (probably complete after 30 minutes at 5°C.); however, the mixture was stirred at 5°C. for 2 hours and the dye precipitated by the addition of ice water. The orange-red powder Compound 13 which was filtered, washed with cold water (5 liters) and vacuum dried was purified by chromatography on a silica gel-cellulose (equal parts by weight) dry packed column by ascending development with a solution of chloroform (8 parts by volume) and methanol (2 parts by volume). A schematic representation of the reactions involved is shown below.

### Step 1



Compound 13 was tested as in Example 12 and found to have a transferred  $\lambda_{max} = 660$  nm, densities: 0.33 (30 sec.), 0.66 (60 sec.) and 1.08 (120 sec.).

A similar compound (Compound 13a) having a sulfonyl ( $-\text{SO}_2\text{NH}_2$ ) radical in place of the sulfo ( $-\text{SO}_3\text{H}$ ) radical on the nitrophenyl ring was prepared and tested as in Example 12. This compound was found to have a transferred  $\lambda_{\text{max}} = 640$  nm,  $D_{\text{max}} = 0.82$ , densities: .53 (30 seconds), 0.71 (60 seconds), and 0.82 (120 seconds).

A similar compound (Compound 13b) having a methylsulfonyl ( $-\text{SO}_2\text{CH}_3$ ) radical in place of the sulfo radical on the nitrophenyl ring was prepared and tested as in Example 12. This compound was found to have a transferred  $\lambda_{\text{max}} = 640$ ,  $D_{\text{max}} = 2.03$ , densities: .85 (30 seconds), 1.40 (60 seconds) and 2.03 (120 seconds).

A similar compound (Compound 13c) having an isopropylsulfonyl radical in place of the sulfo radical on the nitrophenyl ring also gave good results.

### EXAMPLE 15

An image dye-providing compound of the following structure was prepared (Compound 14).



The above compound in diethylauramide solvent was coated as a dispersion in gelatin on polyester support. The layer contained 7.1, 14, and 21 mg/dm<sup>2</sup> of compound, solvent, and gelatin, respectively. A second layer contained a gelatino-silver bromoiodide emulsion with 11 mg/dm<sup>2</sup> of silver and 22 mg/dm<sup>2</sup> of gelatin. The coating was exposed, dipped in the processing composition below for 30 seconds and laminated for varying times with a receiving element containing a mordant layer of poly-4-vinylpyridine and polyvinyl alcohol on a paper support. The processing solution contained (G./liter of solution in water) potassium hydroxide (50), potassium bromide (40), N-benzyl- $\alpha$ -picolinium bromide (20), benzotriazole (20) and sodium sulfate (50). Upon delamination of separate samples after 30, 60, and 120 seconds, respectively, reflection densities of 1.20, 1.55, and 1.80 were measured on the receiver.

**EXAMPLE 16 - Preparation of Compounds 15-21**

Compound 12 of Example 13 is esterified with acetyl chloride in dry acetone using one equivalent of pyridine as the hydrogen chloride acceptor. Compound 15 is similar to Compound 12 of Example 13 only the hydroxy radical in the para position (relative to the point of attachment of the azo linkage) of the naphthalene nucleus is replaced with  $-\text{OCOCH}_3$ . Compound 16 is prepared in a similar manner only using propionyl chloride in the esterification process.

These compounds are tested as in Example 12 with the following results: Compound 15:  $\lambda_{\text{max}}$  of transferred image 640 nm, densities 1.36 (30 sec.), 2.11 (60 sec.), 2.7 (120 sec.); Compound 16:  $\lambda_{\text{max}}$  of transferred image 640 nm, densities 1.20 (30 sec.), 1.95 (60 sec.) and 2.4 (120 sec.).

In a like manner, the hydroxy group in the para position relative to the point of attachment of the azo linkage of the naphthalene nucleus on Compound 12 is replaced with the following groups and tested as in Example 12 with the following results:

| Compound | Group | λ Max<br>(nm.) | D Max | Density of Dye Transfer Image |         |          |
|----------|-------|----------------|-------|-------------------------------|---------|----------|
|          |       |                |       | 30 sec.                       | 60 sec. | 120 sec. |
| 17       |       | 640            | 2.3   | .77                           | 1.46    | 2.3      |
| 18       |       | 640            | 2.0   | .70                           | 1.26    | 2.0      |
| 19       |       | 640            | 2.9   | 1.41                          | 2.4     | 2.9      |
| 20       |       | 640            | 1.18  | .50                           | .77     | 1.18     |
| 21       |       | 640            | —     | .26                           | .47     | .79      |

## EXAMPLE 17

Dyes such as those released from the previously discussed carriers (Car-) during alkaline processing were prepared and dissolved in 30 ml. of a 0.5N sodium hydroxide solution containing 30 g./l. of hydroxyethyl-

5 cellulose. Each solution was spread between a cellulose acetate cover sheet and a receiving element so that the alkaline dye composition was 0.1 mm thick. The receiving element was as described in Example 12 only having an additional layer of gelatin (43 mg/dm<sup>2</sup>)

30 coated over the carbon-gelatin layer. The spectra of the dyes when adsorbed to the mordant were determined as in Example 12. The following Table II shows the general formula of the dyes tested and the results obtained.

Table II

| Dye No. | D                                                       | E                                | M <sup>1</sup>                    | Q <sup>1</sup>        | λ <sub>max</sub> |
|---------|---------------------------------------------------------|----------------------------------|-----------------------------------|-----------------------|------------------|
| 1       | H                                                       | H                                | 5-SO <sub>2</sub> NH <sub>2</sub> | H                     | 610              |
| 2       | SO <sub>2</sub> CH <sub>3</sub>                         | H                                | 5-SO <sub>2</sub> NH <sub>2</sub> | H                     | 634              |
| 3       | SO <sub>2</sub> CH <sub>3</sub>                         | H                                | 6-SO <sub>2</sub> NH <sub>2</sub> | H                     | 639              |
| 4       | SO <sub>2</sub> CH <sub>3</sub>                         | H                                | 7-SO <sub>2</sub> NH <sub>2</sub> | H                     | 630              |
| 5       | SO <sub>2</sub> CH <sub>3</sub>                         | H                                | 8-SO <sub>2</sub> NH <sub>2</sub> | H                     | 616              |
| 6       | SO <sub>2</sub> CH <sub>3</sub>                         | H                                | 5-J <sub>1</sub> *                | H                     | 630              |
| 7       | SO <sub>2</sub> CH <sub>3</sub>                         | H                                | 6-J <sub>1</sub> *                | H                     | 640              |
| 8       | H                                                       | H                                | 6-SO <sub>2</sub> NH <sub>2</sub> | H                     | 612              |
| 9       | Cl                                                      | H                                | 6-SO <sub>2</sub> NH <sub>2</sub> | H                     | 625              |
| 10      | Br                                                      | H                                | 6-SO <sub>2</sub> NH <sub>2</sub> | H                     | 634              |
| 11      | CN                                                      | H                                | 6-SO <sub>2</sub> NH <sub>2</sub> | H                     | 636              |
| 12      | CF <sub>3</sub>                                         | H                                | 6-SO <sub>2</sub> NH <sub>2</sub> | H                     | 637              |
| 13      | NO <sub>2</sub>                                         | H                                | 6-SO <sub>2</sub> NH <sub>2</sub> | H                     | 638              |
| 14      | OCH <sub>3</sub>                                        | H                                | 6-SO <sub>2</sub> NH <sub>2</sub> | H                     | 625              |
| 15      | CH <sub>3</sub>                                         | H                                | 6-SO <sub>2</sub> NH <sub>2</sub> | H                     | 606              |
| 16      | SO <sub>3</sub> Na                                      | H                                | 6-SO <sub>2</sub> NH <sub>2</sub> | H                     | 617              |
| 17      | SO <sub>2</sub> NHC <sub>2</sub> H <sub>5</sub>         | H                                | 6-SO <sub>2</sub> NH <sub>2</sub> | H                     | 633              |
| 18      | —NO <sub>2</sub>                                        | —SO <sub>2</sub> NH <sub>2</sub> | 6-SO <sub>2</sub> NH <sub>2</sub> | H                     | 632              |
| 19      | Cl                                                      | NO <sub>2</sub>                  | 6-SO <sub>2</sub> NH <sub>2</sub> | H                     | 645              |
| 20      | Cl                                                      | Cl                               | 6-SO <sub>2</sub> NH <sub>2</sub> | H                     | 630              |
| 21      | —CN                                                     | —NO <sub>2</sub>                 | 6-SO <sub>2</sub> NH <sub>2</sub> | H                     | 621              |
| 22      | —SO <sub>2</sub> NH(CH <sub>2</sub> ) <sub>2</sub> COOH | H                                | 6-SO <sub>2</sub> NH <sub>2</sub> | H                     | 639              |
| 23      | Cl                                                      | —NO <sub>2</sub>                 | 6-J <sub>1</sub> *                | H                     | 653              |
| 24      | Cl                                                      | H                                | 5-SO <sub>2</sub> NH <sub>2</sub> | H                     | 633              |
| 25      | CN                                                      | H                                | 5-SO <sub>2</sub> NH <sub>2</sub> | H                     | 633              |
| 26      | NO <sub>2</sub>                                         | H                                | 5-SO <sub>2</sub> NH <sub>2</sub> | H                     | 630              |
| 27      | SO <sub>2</sub> CH <sub>3</sub>                         | H                                | 5-SO <sub>2</sub> NH <sub>2</sub> | 8-NHCOCH <sub>3</sub> | 645              |
| 28      | SO <sub>2</sub> CH <sub>3</sub>                         | H                                | 6-SO <sub>2</sub> NH <sub>2</sub> | 8-NHCOCH <sub>3</sub> | 615              |
| 29      | NO <sub>2</sub>                                         | Cl                               | 6-SO <sub>2</sub> NH <sub>2</sub> | 8-NHCOCH <sub>3</sub> | 660              |
| 30      | Cl                                                      | H                                | 5-SO <sub>2</sub> NH <sub>2</sub> | 8-NHCOCH <sub>3</sub> | 610              |
| 31      | H                                                       | H                                | 5-SO <sub>2</sub> NH <sub>2</sub> | 8-NHCOCH <sub>3</sub> | 603              |
| 32      | CN                                                      | H                                | 5-SO <sub>2</sub> NH <sub>2</sub> | 8-NHCOCH <sub>3</sub> | 625              |



Table II-continued



| Dye No. | D                                                               | E               | M¹                  | Q¹                    | λ <sub>max</sub> |
|---------|-----------------------------------------------------------------|-----------------|---------------------|-----------------------|------------------|
| 33      | SO <sub>2</sub> CH <sub>3</sub>                                 | H               | 5-J <sub>1</sub> *  | 8-NHCOCH <sub>3</sub> | 650              |
| 34      | SO <sub>2</sub> CH <sub>3</sub>                                 | H               | 6-J <sub>1</sub> *  | 8-NHCOCH <sub>3</sub> | 669              |
| 35      | SO <sub>2</sub> NHC <sub>6</sub> H <sub>5</sub>                 | H               | H                   | 8-NHCOCH <sub>3</sub> | 625              |
| 36      | SO <sub>2</sub> CH <sub>3</sub>                                 | H               | 5-SO <sub>2</sub> H | 5-J <sub>2</sub> *    | 633              |
| 37      | SO <sub>2</sub> CH <sub>3</sub>                                 | Cl              | H                   | 5-J <sub>2</sub> *    | 640              |
| 38      | SO <sub>2</sub> C <sub>6</sub> H <sub>5</sub>                   | H               | H                   | 5-J <sub>2</sub> *    | 640              |
| 39      | SO <sub>2</sub> (CH <sub>2</sub> ) <sub>3</sub> CH <sub>3</sub> | H               | H                   | 5-J <sub>2</sub> *    | 640              |
| 40      | SO <sub>2</sub> (CH <sub>2</sub> ) <sub>5</sub> CH <sub>3</sub> | H               | H                   | 5-J <sub>2</sub> *    | 640              |
| 41      | SO <sub>2</sub> CH <sub>2</sub> C <sub>6</sub> H <sub>5</sub>   | H               | H                   | 5-J <sub>2</sub> *    | 645              |
| 42      | Cl                                                              | H               | H                   | 5-J <sub>2</sub> *    | 660              |
| 43      | CF <sub>3</sub>                                                 | H               | H                   | 5-J <sub>2</sub> *    | 652              |
| 44      | Br                                                              | H               | H                   | 5-J <sub>2</sub> *    | 657              |
| 45      | CN                                                              | H               | H                   | 5-J <sub>2</sub> *    | 638              |
| 46      | SO <sub>3</sub> C <sub>6</sub> H <sub>5</sub>                   | H               | H                   | 5-J <sub>2</sub> *    | 657              |
| 47      | Cl                                                              | NO <sub>2</sub> | H                   | 5-J <sub>2</sub> *    | 645              |
| 48      | COOH                                                            | H               | H                   | 5-J <sub>2</sub> *    | —                |

\*J<sub>1</sub> = SO<sub>2</sub>NH—C<sub>6</sub>H<sub>4</sub>(m)—SO<sub>2</sub>NH<sub>2</sub>

\*J<sub>2</sub> = NHSO<sub>2</sub>—C<sub>6</sub>H<sub>4</sub>(m)—SO<sub>2</sub>NH<sub>2</sub>

#### EXAMPLE 18

An integral multicolor photosensitive element is prepared by coating the following layers in the order recited on a transparent cellulose acetate film support:

1. image-receiving layer of copoly[styrene-N-benzyl-N,N-dimethyl-N-(3-maleimidopropyl)ammonium chloride] (200 mg./ft.<sup>2</sup>) and gelatin (100 mg./ft.<sup>2</sup>);
2. reflecting layer of titanium dioxide (2000 mg./ft.<sup>2</sup>) and gelatin (200 mg./ft.<sup>2</sup>);
3. opaque layer of carbon black (250 mg./ft.<sup>2</sup>) and gelatin (312 mg./ft.<sup>2</sup>);
4. cyan image dye-providing Compound 12 prepared in Example 13 (65 mg./ft.<sup>2</sup>) and gelatin (100 mg./ft.<sup>2</sup>);
5. red-sensitive, internal-image gelatin-silver chlorobromide emulsion (100 mg. gelatin/ft.<sup>2</sup> and 125 mg. silver/ft.<sup>2</sup>), 2,5-di-sec-dodecylhydroquinone (25 mg./ft.<sup>2</sup>) and nucleating agent formyl-4-methylphenylhydrazine (1 g./mole of silver);
6. interlayer of gelatin (100 mg./ft.<sup>2</sup>) and 2,5-di-sec-dodecylhydroquinone (50 mg./ft.<sup>2</sup>);
7. magenta image dye-providing compound (150 mg./ft.<sup>2</sup>) having the formula



and gelatin (175 mg./ft.<sup>2</sup>);

8. green-sensitive, internal-image gelatin-silver chlorobromide emulsion (125 mg. gelatin/ft.<sup>2</sup> and 150 mg. silver/ft.<sup>2</sup>), 2,5-di-sec-dodecylhydroquinone (50 mg./ft.<sup>2</sup>) and nucleating agent formyl-4-methylphenylhydrazine (1 g./mole of silver);

9. interlayer of gelatin (100 mg./ft.<sup>2</sup>) and 2,5-di-sec-dodecylhydroquinone (50 mg./ft.<sup>2</sup>);

10. yellow image dye-providing compound (100 mg./ft.<sup>2</sup>) having the formula



and gelatin (150 mg./ft.<sup>2</sup>);

11. blue-sensitive internal-image gelatin-silver chlorobromide emulsion (100 mg. gelatin/ft.<sup>2</sup> and 150 mg. silver/ft.<sup>2</sup>), 2,5-di-sec-dodecylhydroquinone (50 mg./ft.<sup>2</sup>) and nucleating agent formyl-4-methylphenylhydrazine (1 g./mole of silver); and

12. overcoat of gelatin (82.5 mg./ft.<sup>2</sup>).

The above silver halide emulsions are direct-positive emulsions having high internal sensitivity and low surface sensitivity of the type described in U.S. Pat. No. 2,592,250.

The above-prepared photosensitive element is then exposed to a graduated-density multicolor test object.

- 60 The following processing composition is employed in a pod and is spread between the photosensitive element and an opaque cellulose acetate sheet by passing the transfer "sandwich" between a pair of juxtaposed pressure rollers:

|                                                  |      |     |
|--------------------------------------------------|------|-----|
| sodium hydroxide                                 | 40   | g.  |
| 4-hydroxymethyl-4-methyl-1-phenyl-3-pyrazolidone | 4    | g.  |
| 5-methylbenzyltriazole                           | 0.1  | g.  |
| potassium iodide                                 | 0.01 | g.  |
| hydroxyethyl cellulose                           | 25   | g.  |
| distilled water to                               | 1000 | ml. |

After 4 minutes, the element is separated from the opaque sheet, subjected to a 1-minute acid rinse, fixed for 4 minutes, washed and dried. The following sensitometric results are obtained.

| Red  | Maximum Density |      | Red  | Minimum Density |      |
|------|-----------------|------|------|-----------------|------|
|      | Green           | Blue |      | Green           | Blue |
| 1.24 | 1.58            | 1.96 | 0.36 | 0.42            | 0.42 |

10

The magenta image dye-providing compound used in this example is prepared as follows:

Predistilled N,N-dimethylformamide (250 ml.) is added to a dried flask containing 22.2 g. (0.05 mol) of  $\alpha$ -[4-hydroxy-3-(2-methoxy-5-sulfamylphenylazo)-1-naphthoxy] propionic acid, 32.5 g. (0.05 mole) of 1-hydroxy-4-m-amino-benzenesulfamyl-N-[ $\Delta$ -(2,4-di-t-amylphenoxy)butyl]-2-naphthamide, and 12.3 g. (0.05 mole) of N-ethoxycarbonyl-2-ethoxy-1,2-dihydroquinoline. The reaction is protected from atmospheric moisture and stirred at room temperature for 4 hours. The reaction is cooled in an ice bath and a solution of 25 g. (0.3 mole) of sodium bicarbonate in 500 ml. of water is added in portions to precipitate an oily solid. An additional 500 ml. of water is added to complete the precipitation. The liquid is decanted from the oily solid and the solid is washed repeatedly with water until the water phase is almost colorless. Any oily solid removed in the original or subsequent decantations is recovered by filtration and thorough washing with water. The oily product is mechanically stirred in 250 ml. of water for 1½ hours to give a crystalline material which is further ground up under water using a mortar and pestle. The resulting slurry is filtered, the solid is washed with water and dried to yield 52 g. (97 percent) of product, m.p. 120°-160°C. The crude product is purified by stirring the product in 300 ml. of acetic acid at room temperature for 1½ hours. The solid is dissolved and reprecipitated. The slurry is filtered and the solid washed with 200 ml. of cold acetic acid followed by 500 ml. of water. The yield of the pure magenta image dye-providing compound is 38 g. (71 percent), m.p. 168°-171°C.,  $\nu_{\text{max}}$  (Dimethylacetamide with triethylamine present) 520-545 nm.

The yellow image dye-providing compound used in this example is prepared as follows:

To a solution of 7.3 g. (0.015 mole) of 1-hydroxy-4-amino-N-[ $\Delta$ -(2,4-di-t-amylphenoxy)butyl]-2-naphthamide in 60 ml. of dye pyridine cooled to 2°C. in an ice bath and stirred in a nitrogen atmosphere are added 6.4 g. (0.016 mole) of 1-phenyl-3-methylcarbamyl-4-(p-chlorosulfonylphenylazo)-5-pyrazolone. The mixture is stirred for 2 hours at room temperature and poured into 1 liter of ice and water containing 75 ml. of hydrochloric acid. The precipitate is collected, dried and recrystallized to give 10.4 g. of the yellow image dye-providing compound.

The photographic elements of this invention can be processed to provide a good positive image in the exposed element by a reversal process. The following example employs an image dye-providing compound adapted for use in the reactions claimed in Hinshaw et al., U.S. Ser. No. 326,628.

An image dye-providing Compound 22 of the following structure is prepared in a manner similar to the methods described in Hinshaw et al., U.S. Ser. No. 326,628.



25

A photographic element is prepared by coating the layers on the support as follows:

1. support;
2. layer containing 40 mg./ft.<sup>2</sup> of the above compound dissolved in 20 mg./ft.<sup>2</sup> of diethyl lauramide, 10 g./ft.<sup>2</sup> of 5-(2-cyanoethylthio)-1-phenyltetrazole dissolved in 30 mg./ft.<sup>2</sup> of tricresyl phosphate, and gelatin at 125 mg./ft.<sup>2</sup>;
3. layer containing a negative silver bromoiodide emulsion coated at 100 mg./ft.<sup>2</sup> based on silver and gelatin at 100 mg./ft.<sup>2</sup>;
4. layer containing galatin at 50 mg./ft.<sup>2</sup>.

A sample of the photographic element is exposed imagewise to a step wedge and processed in Kodak 40 Developer DK-50 at a pH of 9.0 for 15 minutes at 20°C. The element is then washed for 5 minutes, dried, and exposed to room light. The sample is then brought into interfacial contact with an image-receiving element containing a dye mordant with a viscous processing 45 solution inserted between the photographic element and the image-receiving element. The viscous processing solution has the formula:

|    |                                                  |       |
|----|--------------------------------------------------|-------|
| 50 | potassium hydroxide                              | 60 g. |
|    | hydroxyethyl cellulose                           | 30 g. |
|    | 4-hydroxymethyl-4-methyl-1-phenyl-3-pyrazolidone | 3 g.  |
|    | sodium thiosulfate                               | 3 g.  |
|    | potassium bromide                                | 10 g. |
|    | water to 1 liter                                 |       |

55 After 10 minutes the elements are separated. The receiver is washed and dried to provide a good negative image. The photosensitive element is washed, bleached, washed, fixed, washed and dried. A good positive cyan dye image is obtained in this element.

The following compounds within the scope of the invention are prepared and tested as in Example 12. The compounds and results are described in the following Tables III and IV.

Table III



| Compound<br>No. | Car | Density of Dye Transfer Image |         |          |
|-----------------|-----|-------------------------------|---------|----------|
|                 |     | 30 sec.                       | 60 sec. | 120 sec. |
| 23              |     | .78                           | 1.13    | 1.46     |
| 24              |     | 1.31                          | 1.98    | 2.22     |
| 25              |     | 1.09                          | 1.99    | 2.29     |
| 26              |     | 1.14                          | 1.71    | 2.07     |

Table IV



| Compound | R                                                                                   | Density of Dye Transfer Image |         |          |
|----------|-------------------------------------------------------------------------------------|-------------------------------|---------|----------|
|          |                                                                                     | 30 sec.                       | 60 sec. | 120 sec. |
| 27       | CH <sub>3</sub>                                                                     | 1.18                          | 1.57    | 1.96     |
| 28       |  | .54                           | .73     | .93      |

The invention has been described in detail with particular reference to certain preferred embodiments thereof, but it will be understood that variations and modifications can be effected within the spirit and scope of the invention.

**We claim:**

- 55 1. A photosensitive element comprising a support having thereon at least one photosensitive silver halide emulsion layer and one of said layers having associated therewith a cyan image dye-providing compound having a formula as follows:



43

or



5

10

wherein

Car represents a ballasted carrier moiety which, as a function of oxidation of said compound under alkaline conditions, cleaves off from said compound releasing a diffusible dye;

X represents a bivalent linking group of the formula  $-R^2-L_n-R^2_p$ , where each  $R^2$  can be the same or different and each represents an alkylene radical having 1 to about 8 carbon atoms; a phenylene radical; or a phenylene radical substituted with chloro, bromo, cyano, nitro, methoxy, methyl, carboxy or sulfo; L represents a bivalent radical selected from oxy, carbonyl, carboxamido, carbamoyl, sulfonamido, sulfamoyl, sulfinyl or sulfonyl;  $n$  is an integer having a value of 0 or 1;  $p$  is 1 when  $n$  equals 1 and  $p$  is 1 or 0 when  $n$  equals 0, provided that when  $p$  is 1 the carbon content of the sum of both  $R^2$  radicals does not exceed 14 carbon atoms;

R represents a hydrogen atom, or an alkyl radical having 1 to about 6 carbon atoms;

J represents a bivalent radical selected from sulfonyl or carbonyl;

$m$  and  $q$  each represent an integer having a value of 0 or 1;

Q represents a hydrogen atom, a hydroxy radical or a radical having the formula  $-NHCOR^3$  or  $-NHSO_2R^3$  wherein  $R^3$  is an alkyl radical having 1 to about 6 carbon atoms, an alkyl radical having 1 to about 4 carbon atoms substituted with hydroxy, cyano, sulfamoyl, carboxy or sulfo; benzyl phenyl, or a phenyl radical substituted with carboxy, chloro, methyl, methoxy or sulfamoyl;

G represents a hydroxy radical, a salt thereof, or a hydrolyzable acyloxy group having the formula:



50

wherein  $R^4$  is an alkyl radical having 1 to about 18 carbon atoms, phenyl or phenyl substituted with chloro or nitro;

D represents a halogen atom, a cyano radical, a nitro radical, a trifluoromethyl radical, an alkyl radical having 1 to about 6 carbon atoms, an alkoxy radical having 1 to about 6 carbon atoms, a carboxy radical, a carboxylic acid ester having the formula  $-\text{COOR}^4$  wherein  $R^4$  is as described previously, a fluorosulfonyl radical, a  $-\text{SO}_3$ -phenyl radical or a  $-\text{SO}_3$ -phenyl radical substituted with hydroxy, chloro, carboxy, sulfamoyl, methyl or methoxy; a sulfo radical, a sulfamoyl radical having the formula  $-\text{SO}_2\text{NR}^5\text{R}^6$  wherein  $R^5$  represents hydrogen or an alkyl group having 1 to about 6 carbon atoms and  $R^6$  represents hydrogen, an alkyl radical having 1 to about 6 carbon atoms, an alkyl radical having 1 to about 4 carbon atoms substituted with hydroxy, cyano, sulfamoyl, carboxy or sulfo; a benzyl

44

radical, a phenyl radical, a phenyl radical substituted with hydroxy, sulfonyl, sulfamoyl, carboxy or sulfo; an alkyl carbonyl radical having 1 to about 8 carbon atoms, or a phenyl carbonyl radical, with the proviso that the carbon content of the sum of  $R^5$  and  $R^6$  not exceed 14 carbon atoms; a carbamoyl radical having the formula  $-\text{CON}(\text{R}^5)_2$  wherein each  $R^5$  can be the same or different and is as described previously; an alkylsulfonyl radical having 1 to about 8 carbon atoms; an alkylsulfonyl radical having 1 to about 6 carbon atoms substituted with hydroxy, phenyl, cyano, sulfamoyl, carboxy or sulfo; a phenylsulfonyl radical; a phenylsulfonyl radical substituted with hydroxy, sulfonyl, sulfamoyl, carboxy or sulfo; or D can represent a substituent having the formula  $\text{Car}-[\text{X}-(\text{NR}-\text{J})_q]_m$  or  $\text{Car}-\text{X}-\text{J}$ , provided that the  $\text{Car}-[\text{X}-(\text{NR}-\text{J})_q]_m$ -substituent on the naphthalene nucleus of Formula I is replaced by an M group or the  $\text{Car}-\text{X}-\text{J}-\text{NH}$ -substituent on the naphthalene nucleus of Formula II is replaced by a Q group wherein Car, X, J, R, q and m are as described previously.

E represents a hydrogen atom, a halogen atom, a nitro radical, a cyano radical or a trifluoromethyl radical;

M represents a hydrogen atom, a carboxy radical, a carboxylic acid ester having the formula  $-\text{COOR}^4$  wherein  $R^4$  is as described previously, a sulfo radical, a sulfamoyl radical having the formula  $-\text{SO}_2\text{NR}^5\text{R}^6$ , a carbamoyl radical having the formula  $-\text{CON}(\text{R}^5)_2$  wherein  $R^5$  and  $R^6$  are as described previously, an alkylsulfonyl radical having 1 to about 8 carbon atoms; an alkylsulfonyl radical having 1 to about 6 carbon atoms substituted with cyano or hydroxy; a phenylsulfonyl radical or a phenylsulfonyl radical substituted with sulfamoyl, carboxy, fluorosulfonyl or methoxy; with the proviso that there be no more than one sulfo radical and no more than one carboxy radical present in said compound.

2. A photosensitive element as described in claim 1 wherein  $n$  and  $p$  each have a value of 0.

3. A photosensitive element as described in claim 1 wherein  $m$  has a value of 0.

4. A photosensitive element as described in claim 1 wherein G is a hydroxy radical.

5. A photosensitive element as described in claim 1 wherein E represents a hydrogen atom, a halogen atom or a nitro radical; and M represents a hydrogen atom or a sulfamoyl radical as described in claim 1.

6. A photosensitive element as described in claim 1 wherein

$R^2$  represents an alkylene radical having 1 to about 4 carbon atoms, phenylene or phenylenes substituted with carboxy, chloro, methyl or methoxy;

L represents sulfamoyl, sulfonamido, carbamoyl or carboxamido;

R represents hydrogen;

$q$  is an integer having a value of 1;

$m$  is an integer having a value of 0 or 1;

Q represents hydrogen, hydroxy,  $-NHCOR^3$  or  $-NHSO_2R^3$  wherein  $R^3$  represents an alkyl radical having 1 to about 4 carbon atoms; an alkyl radical having 1 to about 4 carbon atoms substituted with hydroxy, cyano, sulfamoyl, carboxy or sulfo; benzyl, phenyl or phenyl substituted with carboxy, chloro, methyl, methoxy or sulfamoyl;

D represents chloro, fluoro, bromo, cyano, trifluoromethyl, nitro, fluorosulfonyl, alkylsulfonyl having 1 to about 6 carbon atoms, alkylsulfonyl having 1 to

about 6 carbon atoms substituted with hydroxy, phenyl, cyano, sulfamoyl, carboxy or sulfo; phenylsulfonyl; phenylsulfonyl substituted with hydroxy, sulfamoyl, fluorosulfonyl, carboxy or sulfo; a sulfamoyl radical having the formula  $-\text{SO}_2\text{NHR}^6$  wherein  $\text{R}^6$  is hydrogen, an alkyl radical having 1 to about 4 carbon atoms, or an alkyl radical having 1 to about 4 carbon atoms substituted with hydroxy, cyano, sulfamoyl, carboxy or sulfo; benzyl, phenyl or phenyl substituted with hydroxy, sulfonyl, sulfamoyl, carboxy or sulfo; a carbamoyl radical having the formula  $-\text{CON}(\text{R}^5)_2$  wherein  $\text{R}^5$  is hydrogen or methyl, and

D can represent a substituent having the formula  $\text{Car-}[\text{X-(NR-J)}_q]_m$  or  $\text{Car-X-J-}$ , provided that the  $\text{Car-}[\text{X-(NR-J)}_q]_m$ - substituent on the naphthalene nucleus of Formula I is replaced by an M group or the  $\text{Car-X-J-NH}$  substituent on the naphthalene nucleus of Formula II is replaced by a Q group wherein Car, X, J, R, q and m are as described previously;

E represents hydrogen, fluoro, or chloro; and M represents hydrogen or a sulfamoyl radical of the formula  $-\text{SO}_2\text{NHR}^6$  wherein  $\text{R}^6$  is hydrogen; an alkyl radical of 1 to about 4 carbon atoms; an alkyl radical having 1 to about 6 carbon atoms substituted with hydroxy, cyano, sulfamoyl, carboxy, or sulfo; benzyl, phenyl or phenyl substituted with hydroxy, sulfamoyl, carboxy or sulfo.

7. A photosensitive element as described in claim 6 wherein n and p each have a value of 0.

8. A photosensitive element as described in claim 6 wherein m has a value of 0.

9. A photosensitive element as described in claim 6 wherein G is a hydroxy radical.

10. A photosensitive element as described in claim 6 wherein E represents a hydrogen atom, a halogen atom or nitro radical; and M represents a hydrogen atom.

11. A photosensitive element as described in claim 6 wherein the  $\text{Car-X-J-NH}$ - substituent in Formula II is in the 5-position on the naphthalene nucleus relative to G; and the  $\text{Car-}[\text{X-(NR-J)}_q]_m$ - substituent in Formula I is in the 5- or 6-position on the naphthalene nucleus relative to G;

$\text{R}^2$  represents an alkylene radical having 1 to about 4 carbon atoms, or phenylene;

L represents sulfamoyl or sulfonamido;

J represents sulfonyl;

Q is in the 8-position relative to G and represents hydrogen, hydroxy,  $-\text{NHSO}_2\text{R}^3$  or  $-\text{NHCOCH}_3$ ;

G represents hydroxy, a photographically inactive ammonium salt thereof, or a hydrolyzable acyloxy group having the formula:



wherein  $\text{R}^4$  is an alkyl radical having 1 to about 18 carbon atoms, phenyl or phenyl substituted with chloro or nitro;

D represents chloro, bromo, cyano, trifluoromethyl, nitro, alkylsulfonyl having 1 to about 6 carbon atoms, or benzylsulfonyl;

E represents hydrogen; and

M represents hydrogen.

12. A photosensitive element as described in claim 11 wherein X represents



5 G represents hydroxy or a hydrolyzable acyloxy group; and

D represents an alkylsulfonyl radical having 1 to about 4 carbon atoms.

13. A photosensitive element comprising a support having thereon at least one photosensitive silver halide emulsion layer and one of said layers having associated therewith a cyan image dye-providing compound having a formula as follows:

15

I.



20

II.



wherein

40 Ball represents an organic ballasting group of such size and configuration as to render said compound nondiffusible during development in an alkaline processing composition;

Y represents the carbon atoms necessary to complete a benzene or naphthalene nucleus;

X represents a bivalent linking group of the formula  $-\text{R}^2-\text{L}_n-\text{R}^2-$  where each  $\text{R}^2$  can be the same or different and each represents an alkylene radical having 1 to about 8 carbon atoms; a phenylene radical; or a phenylene radical substituted with chloro, bromo, cyano, nitro, methoxy, methyl, carboxy or sulfo; L represents a bivalent radical selected from oxy, carbonyl, carboxamido, carbamoyl, sulfonamido, sulfamoyl, sulfinyl or sulfonyl; n is an integer having a value of 0 or 1; p is 1 when n equals 1 and p is 1 or 0 when n equals 0, provided that when p is 1 the carbon content of the sum of both  $\text{R}^2$  radicals does not exceed 14 carbon atoms;

R represents a hydrogen atom, or an alkyl radical having 1 to about 6 carbon atoms;

J represents a bivalent radical selected from sulfonyl or carbonyl;

m and q each represent an integer having a value of 0 or 1;

Q represents a hydrogen atom, a hydroxy radical or a radical having the formula  $-\text{NHCOR}^3$  or  $-\text{NHSO}_2\text{R}^3$  wherein  $\text{R}^3$  is an alkyl radical having 1 to about 6 carbon atoms, an alkyl radical having 1 to about 4

carbon atoms substituted with hydroxy, cyano, sulfamoyl, carboxy or sulfo; benzyl, phenyl, or a phenyl radical substituted with carboxy, chloro, methyl, methoxy or sulfamoyl; G represents a hydroxy radical, a salt thereof, or a hydrolyzable acyloxy group having the formula:



wherein  $\text{R}^4$  is an alkyl radical having 1 to about 18 carbon atoms, phenyl or phenyl substituted with chloro or nitro;

D represents a halogen atom, a cyano radical, a nitro radical, a trifluoromethyl radical, an alkyl radical having 1 to about 6 carbon atoms, an alkoxy radical having 1 to about 6 carbon atoms, a carboxy radical, a carboxylic acid ester having the formula  $-\text{COOR}^4$  wherein  $\text{R}^4$  is as described previously, a fluorosulfonyl radical, a  $-\text{SO}_3$ -phenyl radical or a  $-\text{SO}_3$ -phenyl radical substituted with hydroxy, chloro, carboxy, sulfamoyl, methyl or methoxy; a sulfo radical, a sulfamoyl radical having the formula  $-\text{SO}_2\text{NR}^5\text{R}^6$  wherein  $\text{R}^5$  represents hydrogen or an alkyl group having 1 to about 6 carbon atoms and  $\text{R}^6$  represents hydrogen, an alkyl radical having 1 to about 6 carbon atoms, an alkyl radical having 1 to about 4 carbon atoms substituted with hydroxy, cyano, sulfamoyl, carboxy or sulfo; a benzyl radical, a phenyl radical, a phenyl radical substituted with hydroxy, sulfonyl, sulfamoyl, carboxy or sulfo; an alkyl carbonyl radical having 1 to about 8 carbon atoms, or a phenyl carbonyl radical, with the proviso that the carbon content of the sum of  $\text{R}^5$  and  $\text{R}^6$  not exceed 14 carbon atoms; a carbamoyl radical of the formula  $-\text{CON}(\text{R}^5)_2$  wherein each  $\text{R}^5$  can be the same or different and is as described previously; an alkylsulfonyl radical having 1 to about 8 carbon atoms; an alkylsulfonyl radical having 1 to about 6 carbon atoms substituted with hydroxy, phenyl, cyano, sulfamoyl, carboxy or sulfo; a phenylsulfonyl radical; a phenylsulfonyl radical substituted with hydroxy, sulfonyl, sulfamoyl, carboxy or sulfo; or D can represent a substituent having the formula



provided that the



substituent on the naphthalene nucleus of Formula I is replaced by an M group or the

substituent on the naphthalene nucleus of Formula II is replaced by a Q group wherein Car, X, J, R, q and m are as described previously.

E represents a hydrogen atom, a halogen atom, a nitro radical, a cyano radical or a trifluoromethyl radical;

M represents a hydrogen atom, a carboxy radical, a carboxylic acid ester having the formula  $-\text{COOR}^4$  wherein  $\text{R}^4$  is as described previously, a sulfo radical, a sulfamoyl radical having the formula  $-\text{SO}_2\text{NR}^5\text{R}^6$ , a carbamoyl radical having the formula  $-\text{CON}(\text{R}^5)_2$  wherein  $\text{R}^5$  and  $\text{R}^6$  are as described previously, an alkylsulfonyl radical having 1 to about 8 carbon atoms; an alkylsulfonyl radical having 1 to about 6 carbon atoms substituted with cyano or hydroxy; a phenylsulfonyl radical or a phenylsulfonyl radical substituted with sulfamoyl, carboxy, fluorosulfonyl or methoxy;

with the proviso that there be no more than one sulfo radical and no more than one carboxy radical present in said compound.

14. A photosensitive element as described in claim

13 wherein

$\text{R}^2$  represents an alkylene radical having 1 to about 4 carbon atoms, phenylene or phethylene substituted with carboxy, chloro, methyl or methoxy;

L represents sulfamoyl, sulfonamido, carbamoyl, or carboxamido;

R represents hydrogen;

q is an integer having a value of 1;

m is an integer having a value of 0 or 1;

Q represents hydrogen, hydroxy,  $-\text{NHCOR}^3$  or  $-\text{NHSO}_2\text{R}^3$  wherein  $\text{R}^3$  represents an alkyl radical having 1 to about 4 carbon atoms, an alkyl radical having 1 to about 4 carbon atoms substituted with hydroxy, cyano, sulfamoyl, carboxy or sulfo; benzyl, phenyl, phenyl substituted with carboxy, chloro, methyl, methoxy or sulfamoyl;

D represents chloro; fluoro; bromo; cyano; trifluoromethyl; nitro; fluorosulfonyl; alkylsulfonyl having 1 to about 6 carbon atoms; alkylsulfonyl having 1 to about 6 carbon atoms substituted with hydroxy, phenyl, cyano, sulfamoyl, carboxy or sulfo; phenylsulfonyl; phenylsulfonyl substituted with hydroxy, sulfamoyl, fluorosulfonyl, carboxy or sulfo; a sulfamoyl radical having the formula  $-\text{SO}_2\text{NHR}^6$  wherein  $\text{R}^6$  is hydrogen, an alkyl radical having 1 to about 4 carbon atoms or an alkyl radical having 1 to about 4 carbon atoms substituted with hydroxy, cyano, sulfamoyl, carboxy, or sulfo; benzyl, phenyl or phenyl substituted with hydroxy, sulfonyl, sulfamoyl, carboxy or sulfo; a carbamoyl radical having the formula  $-\text{CON}(\text{R}^5)_2$  wherein  $\text{R}^5$  is hydrogen or methyl, and

D can represent a substituent having the formula



provided that the



substituent on the naphthalene nucleus of Formula I is replaced by an M group or the



substituent on the naphthalene nucleus of Formula II is replaced by a Q group wherein Y, Ball, X, R, J, q and m are as described previously;

E represents hydrogen, fluoro or chloro; and  
M represents hydrogen or a sulfamoyl radical of the formula  $-\text{SO}_2\text{NHR}^6$  wherein  $\text{R}^6$  is hydrogen; an alkyl radical of 1 to about 4 carbon atoms; an alkyl radical having 1 to about 4 carbon atoms substituted with hydroxy, cyano, sulfamoyl, carboxy, or sulfo; benzyl, phenyl or phenyl substituted with hydroxy, sulfamoyl, carboxy or sulfo.

15. A photosensitive element as described in claim 14 wherein n and p each have a value of 0.

16. A photosensitive element as described in claim 14 wherein m has a value of 0.

17. A photosensitive element as described in claim 14 wherein G is a hydroxy radical.

18. A photosensitive element as described in claim 14 wherein E represents a hydrogen atom; and M represents a hydrogen atom.

19. A photosensitive element as described in claim 14 wherein the



containing substituent on the naphthalene nucleus is in the 5- or 6-position relative to G in Formula I and in the 5-position relative to G in Formula II;

Y represents the atoms necessary to complete a naphthalene nucleus;

$\text{R}^2$  represents an alkylene radical having 1 to about 4 carbon atoms, or phenyl;

L represents sulfamoyl or sulfonamido;

J represents sulfonyl;

Q is in the 8-position relative to G and represents hydrogen, hydroxy,  $-\text{NHSO}_2\text{CH}_3$ , or  $-\text{NH-COCH}_3$ ;

G represents hydroxy, a photographically inactive ammonium salt thereof, or a hydrolyzable acyloxy group having the formula



5 wherein  $\text{R}^4$  is an alkyl having 1 to about 18 carbon atoms, phenyl or phenyl substituted with chloro or nitro;

D represents chloro, bromo, cyano, trifluoromethyl, nitro, alkylsulfonyl having 1 to about 6 carbon atoms or benzylsulfonyl;

E represents hydrogen; and

M represents hydrogen.

20. A photosensitive element as described in claim 19 wherein X represents



20 G represents hydroxy or a hydrolyzable acyloxy group; and

D represents an alkylsulfonyl radical having 1 to about 4 carbon atoms.

21. A photosensitive element as described in claim 19 wherein -Ball is linked to the sulfonamidonaphthol nucleus through a bivalent



30 moiety.

22. A photosensitive element as described in claim 20 wherein -Ball represents



40 and is in the 2-position relative to the hydroxy group.

23. A photosensitive element as described in claim 1 wherein said cyan image dye-providing compound is contained in a layer contiguous to the silver halide emulsion layer.

45 24. A photosensitive element as described in claim 6 wherein said cyan image dye-providing compound is contained in a layer contiguous to the silver halide emulsion layer.

25. A photosensitive element as described in claim 50 11 wherein said cyan image dye-providing compound is contained in a layer contiguous to the silver halide emulsion layer.

26. A photosensitive element as described in claim 12 wherein said cyan image dye-providing compound is contained in a layer contiguous to the silver halide emulsion layer.

55 27. A photosensitive element as described in claim 13 wherein said cyan image dye-providing compound is contained in a layer contiguous to the silver halide emulsion layer.

60 28. A photosensitive element as described in claim 14 wherein said cyan image dye-providing compound is contained in a layer contiguous to the silver halide emulsion layer.

65 29. A photosensitive element as described in claim 15 wherein said cyan image dye-providing compound is contained in a layer contiguous to the silver halide emulsion layer.

30. A photosensitive element as described in claim 16 wherein said cyan image dye-providing compound is contained in a layer contiguous to the silver halide emulsion layer.

31. A photosensitive element as described in claim 19 wherein said cyan image dye-providing compound is contained in a layer contiguous to the silver halide emulsion layer.

32. A photosensitive element as described in claim 20 wherein said cyan image dye-providing compound is contained in a layer contiguous to the silver halide emulsion layer.

33. A photosensitive element as described in claim 21 wherein said cyan image dye-providing compound is contained in a layer contiguous to the silver halide emulsion layer.

34. A photosensitive element as described in claim 22 wherein said cyan image dye-providing compound is contained in a layer contiguous to the silver halide emulsion layer.

35. A photosensitive element comprising a support having thereon a layer containing a red-sensitive silver halide emulsion having associated therewith a cyan image dye-providing material, a layer containing a green-sensitive silver halide emulsion having associated therewith a magenta image dye-providing material, and a layer containing a blue-sensitive silver halide emulsion having associated therewith a yellow image dye-providing material, said cyan image dye-providing material having a formula as follows:



wherein

Car represents a ballasted carrier moiety which, as a function of oxidation of said compound under alkaline conditions, cleaves off from said compound releasing a diffusible dye;

X represents a bivalent linking group of the formula  $-\text{R}^2-\text{L}_n-\text{R}^2-$ , where each  $\text{R}^2$  can be the same or different and each represents an alkylene radical having 1 to about 8 carbon atoms; a phenylene radical; or a phenylene radical substituted with chloro, bromo, cyano, nitro, methoxy, methyl, carboxy or sulfo; L represents a bivalent radical selected from oxy, carbonyl, carboxamido, carbamoyl, sulfonamido, sulfamoyl, sulfinyl or sulfonyl; n is an integer having a value of 0 or 1; p is 1 when n equals 1 and p is 1 or 0 when n equals 0, provided that when p is 1 the carbon content of the sum of both  $\text{R}^2$  radicals does not exceed 14 carbon atoms;

R represents a hydrogen atom, or an alkyl radical having 1 to about 6 carbon atoms;

J represents a bivalent radical selected from sulfonyl or carbonyl;

m and q each represent an integer having a value of 0 or 1;

Q represents a hydrogen atom, a hydroxy radical or a radical having the formula  $-\text{NHCOR}^3$  or  $-\text{NHSO}_2\text{R}^3$  wherein  $\text{R}^3$  is an alkyl radical having 1 to about 6 carbon atoms, an alkyl radical having 1 to about 4 carbon atoms substituted with hydroxy, cyano, sulfamoyl, carboxy or sulfo; benzyl, phenyl, or a phenyl radical substituted with carboxy, chloro, methyl, methoxy or sulfamoyl;

G represents a hydroxy radical, a salt thereof, or a hydrolyzable acyloxy group having the formula:



wherein  $\text{R}^4$  is an alkyl radical having 1 to about 18 carbon atoms, phenyl or phenyl substituted with chloro or nitro;

D represents a halogen atom, a cyano radical, a nitro radical, a trifluoromethyl radical, an alkyl radical having 1 to about 6 carbon atoms, an alkoxy radical having 1 to about 6 carbon atoms, a carboxy radical, a carboxylic acid ester having the formula  $-\text{COOR}^4$  wherein  $\text{R}^4$  is as described previously, a fluorosulfonyl radical, a  $-\text{SO}_3\text{-phenyl}$  radical or a  $-\text{SO}_3\text{-phenyl}$  radical substituted with hydroxy, chloro, carboxy, sulfamoyl, methyl or methoxy; a sulfo radical, a sulfamoyl radical having the formula  $-\text{SO}_2\text{NR}^5\text{R}^6$  wherein  $\text{R}^5$  represents hydrogen or an alkyl group having 1 to about 6 carbon atoms and  $\text{R}^6$  represents hydrogen, an alkyl radical having 1 to about 6 carbon atoms, an alkyl radical having 1 to about 4 carbon atoms substituted with hydroxy, cyano, sulfamoyl, carboxy or sulfo; a benzyl radical, a phenyl radical, a phenyl radical substituted with hydroxy, sulfonyl, sulfamoyl, carboxy or sulfo; an alkyl carbonyl radical having 1 to about 8 carbon atoms, or a phenyl carbonyl radical, with the proviso that the carbon content of the sum of  $\text{R}^5$  and  $\text{R}^6$  not exceed 14 carbon atoms; a carbamoyl radical having the formula  $-\text{CON}(\text{R}^5)_2$  wherein each  $\text{R}^5$  can be the same or different and is as described previously; an alkylsulfonyl radical having 1 to about 8 carbon atoms; an alkylsulfonyl radical having 1 to about 6 carbon atoms substituted with hydroxy, phenyl, cyano, sulfamoyl, carboxy or sulfo; a phenylsulfonyl radical; a phenylsulfonyl radical substituted with hydroxy, sulfonyl, sulfamoyl, carboxy or sulfo; or D can represent a substituent having the formula  $\text{Car}-[\text{X}-(\text{NR}-\text{J})_q]_m$  or  $\text{Car}-\text{X}-\text{J}-$ , provided that the  $\text{Car}-[\text{X}-(\text{NR}-\text{J})_q]_m$  substituent on the naphthalene nucleus of Formula I is replaced by an M group or the  $\text{Car}-\text{X}-\text{J}-$  substituent on the naphthalene nucleus of Formula II is replaced by a Q group wherein Car, X, J, R, q and m are as described previously.

E represents a hydrogen atom, a halogen atom, a nitro radical, a cyano radical or a trifluoromethyl radical;

M represents a hydrogen atom, a carboxy radical, a carboxylic acid ester having the formula  $-\text{COOR}^4$  wherein  $\text{R}^4$  is as described previously, a sulfo radical, a sulfamoyl radical having the formula  $-\text{SO}_2\text{NR}^5\text{R}^6$ , a carbamoyl radical having the formula  $-\text{CON}(\text{R}^5)_2$  wherein  $\text{R}^5$  and  $\text{R}^6$  are as described previously, an alkylsulfonyl radical having 1 to about 8 carbon atoms; an alkylsulfonyl radical having 1 to about 6 carbon atoms substituted with

cyano or hydroxy; a phenylsulfonyl radical or a phenylsulfonyl radical substituted with sulfamoyl, carboxy, fluorosulfonyl or methoxy; with the proviso that there be no more than one sulfo radical and no more than one carboxy radical present in said compound.

36. A photosensitive element as described in claim 35 wherein  $n$  and  $p$  each have a value of 0.

37. A photosensitive element as described in claim 35 wherein  $m$  has a value of 0.

38. A photosensitive element as described in claim 35 wherein G is a hydroxy radical;

E represents a hydrogen atom, a halogen atom or a nitro radical; and M represents a hydrogen atom or a sulfamoyl radical as described in claim 1.

39. A photosensitive element as described in claim 35 wherein

$R^2$  represents an alkylene radical having 1 to about 4 carbon atoms, phenylene or phenoxy substituted with carboxy, chloro, methyl or methoxy;

L represents sulfamoyl, sulfonamido, carbamoyl or carboxamido;

R represents hydrogen;

$q$  is an integer having a value of 1;

$m$  is an integer having a value of 0 or 1;

Q represents hydrogen, hydroxy,  $-\text{NHCOR}^3$  or  $-\text{NHSO}_2\text{R}^3$  wherein  $R^3$  represents an alkyl radical having 1 to about 4 carbon atoms; an alkyl radical having 1 to about 4 carbon atoms substituted with hydroxy, cyano, sulfamoyl, carboxy or sulfo; benzyl, phenyl or phenyl substituted with carboxy, chloro, methyl, methoxy or sulfamoyl;

D represents chloro, fluoro, bromo, cyano, trifluoromethyl, nitro, fluorosulfonyl, alkylsulfonyl having 1 to about 6 carbon atoms, alkylsulfonyl having 1 to about 6 carbon atoms substituted with hydroxy, phenyl, cyano, sulfamoyl, carboxy or sulfo; phenylsulfonyl; phenylsulfonyl substituted with hydroxy, sulfamoyl, fluorosulfonyl, carboxy or sulfo; a sulfamoyl radical having the formula  $-\text{SO}_2\text{NHR}^6$  wherein  $R^6$  is hydrogen, an alkyl radical having 1 to about 4 carbon atoms, or an alkyl radical having 1 to about 4 carbon atoms substituted with hydroxy, cyano, sulfamoyl, carboxy or sulfo; benzyl, phenyl or phenyl substituted with hydroxy, sulfonamido, sulfamoyl, carboxy or sulfo; a carbamoyl radical having the formula  $-\text{CON}(\text{R}^3)_2$  wherein  $R^3$  is hydrogen or methyl, and

D can represent a substituent having the formula  $\text{Car-}[\text{X-}(\text{NR-J})_q]_m-$  or  $\text{Car-X-J-}$ , provided that the  $\text{Car-}[\text{X-}(\text{NR-J})_q]_m-$  substituent on the naphthalene nucleus of Formula I is replaced by an M group or the  $\text{Car-X-J-NH-}$  substituent on the naphthalene nucleus of Formula II is replaced by a Q group wherein Car, X, J, R, q and m are as described previously;

E represents hydrogen, fluoro, or chloro; and

M represents hydrogen or a sulfamoyl radical of the formula  $-\text{SO}_2\text{NHR}^6$  wherein  $R^6$  is hydrogen; an alkyl radical of 1 to about 4 carbon atoms; an alkyl radical having 1 to about 6 carbon atoms substituted with hydroxy, cyano, sulfamoyl, carboxy, or sulfo; benzyl, phenyl or phenyl substituted with hydroxy, sulfamoyl, carboxy or sulfo.

40. A photosensitive element as described in claim 39 wherein  $n$  and  $p$  each have a value of 0.

41. A photosensitive element as described in claim 39 wherein  $m$  has a value of 0.

42. A photosensitive element as described in claim 39 wherein G is a hydroxy radical.

43. A photosensitive element as described in claim 39 wherein E represents a hydrogen atom, a halogen atom or nitro radical; and M represents a hydrogen atom.

44. A photosensitive element as described in claim 39 wherein the  $\text{Car-X-J-NH-}$  substituent in Formula II is in the 5-position on the naphthalene nucleus relative to G; and the  $\text{Car-}[\text{X-}(\text{NR-J})_q]_m-$  substituent in Formula I is in the 5- or 6-position on the naphthalene nucleus relative to G;

$R^2$  represents an alkylene radical having 1 to about 4 carbon atoms or phenylene;

L represents sulfamoyl or sulfonamido;

J represents sulfonyl;

Q is in the 8-position relative to G and represents hydrogen, hydroxy,  $-\text{NHSO}_2\text{R}^3$  or  $-\text{NHOCH}_3$ ;

G represents hydroxy, a photographically inactive ammonium salt thereof, or a hydrolyzable acyloxy group having the formula:



wherein  $R^4$  is an alkyl radical having 1 to about 18 carbon atoms, phenyl or phenyl substituted with chloro or nitro;

D represents chloro, bromo, cyano, trifluoromethyl, nitro, alkylsulfonyl having 1 to about 6 carbon atoms, or benzylsulfonyl;

E represents hydrogen; and

M represents hydrogen.

45. A photosensitive element as described in claim 44 wherein X represents



G represents hydroxy or a hydrolyzable acyloxy group; and

D represents an alkylsulfonyl radical having 1 to about 4 carbon atoms.

46. A photosensitive element comprising a support having thereon a layer containing a red-sensitive silver halide emulsion having associated therewith a cyan image dye-providing material, a layer containing a green-sensitive silver halide emulsion having associated therewith a magenta image dye-providing material, and a layer containing a blue-sensitive silver halide emulsion having associated therewith a yellow image dye-providing material, said cyan image dye-providing material having a formula as follows:

i.



or



wherein

Ball represents an organic ballasting group of such size and configuration as to render said compound nondiffusible during development in an alkaline processing composition;

Y represents the carbon atoms necessary to complete a benzene or naphthalene nucleus:

X represents a bivalent linking group of the formula  $-R^2-L_n-R^2_p-$  where each  $R^2$  can be the same or different and each represents an alkylene radical having 1 to about 8 carbon atoms; a phenylene radical; or a phenylene radical substituted with chloro, bromo, cyano, nitro, methoxy, methyl, carboxy or sulfo; L represents a bivalent radical selected from oxy, carbonyl, carboxamido, carbamoyl, sulfonamido, sulfamoyl, sulfinyl or sulfonyl; n is an integer having a value of 0 or 1; p is 1 when n equals 1 and p is 1 or 0 when n equals 0, provided that when p is 1 the carbon content of the sum of both  $R^2$  radicals does not exceed 14 carbon atoms;

R represents a hydrogen atom, or an alkyl radical having 1 to about 6 carbon atoms;

J represents a bivalent radical selected from sulfonyl or carbonyl;

m and q each represent an integer having a value of 0 or 1;

Q represents a hydrogen atom, a hydroxy radical or a radical having the formula  $\text{-NHCOR}^3$  or  $\text{-HSO}_2\text{R}^3$

wherein  $R^3$  is an alkyl radical having 1 to about 6 carbon atoms, an alkyl radical having 1 to about 4 carbon atoms substituted with hydroxy, cyano, sulfamoyl, carboxy or sulfo; benzyl, phenyl, or a phenyl radical substituted with carboxy, chloro, methyl, methoxy or sulfamoyl;

G represents a hydroxy radical, a salt thereof, or a hydrolyzable acyloxy group having the formula:



wherein R<sup>4</sup> is an alkyl radical having 1 to about 18 carbon atoms, phenyl or phenyl substituted with chloro or nitro;

D represents a halogen atom, a cyano radical, a nitro radical, a trifluoromethyl radical, an alkyl radical having 1 to about 6 carbon atoms, an alkoxy radical having 1 to about 6 carbon atoms, a carboxy radical, a carboxylic acid ester having the formula -COOR<sub>4</sub> wherein R<sub>4</sub> is as described previously, a fluorosulfonyl radical, a -SO<sub>3</sub>-phenyl radical or a -SO<sub>3</sub>-phenyl radical substituted with hydroxy, chloro, carboxy, sulfamoyl, methyl or methoxy; a sulfo radical, a sulfamoyl radical having the formula -SO<sub>2</sub>NR<sup>5</sup>R<sup>6</sup> wherein R<sup>5</sup> represents hydrogen or an alkyl group having 1 to about 6 carbon atoms and R<sup>6</sup> represents hydrogen, an alkyl radical having 1 to about 6 carbon atoms, an alkyl radical having 1 to about 4 carbon atoms substituted with hydroxy, cyano, sulfamoyl, carboxy or sulfo; a benzyl radical, a phenyl

radical, a phenyl radical substituted with hydroxy, sulfonyl, sulfamoyl, carboxy or sulfo; an alkyl carbonyl radical having 1 to about 8 carbon atoms, or a phenyl carbonyl radical, with the proviso that the carbon content of the sum of  $R^5$  and  $R^6$  not exceed 14 carbon atoms; a carbamoyl radical of the formula  $-CON(R^5)_2$ , wherein each  $R^5$  can be the same or different and is as described previously; an alkylsulfonyl radical having 1 to about 8 carbon atoms; an alkylsulfonyl radical having 1 to about 6 carbon atoms substituted with hydroxy, phenyl, cyano, sulfamoyl, carboxy or sulfo; a phenylsulfonyl radical; a phenylsulfonyl radical substituted with hydroxy, sulfonyl, sulfamoyl, carboxy or sulfo; or D can represent a substituent having the formula



provided that the



substituent on the naphthalene nucleus of Formula I is replaced by an M group or the



5 substituent on the naphthalene nucleus of Formula II is replaced by a Q group wherein Car, X, J, R, q and m are as described previously.

E represents a hydrogen atom, a halogen atom, a nitro radical, a cyano radical or a trifluoromethyl radical;

M represents a hydrogen atom, a carboxy radical, a carboxylic acid ester having the formula -COOR<sup>4</sup>, wherein R<sup>4</sup> is as described previously, a sulfo radical, a sulfamoyl radical having the formula -SO<sub>2</sub>NR<sup>5</sup>R<sup>6</sup>, a carbamoyl radical having the formula -CON(R<sub>5</sub>)<sub>2</sub> wherein R<sup>5</sup> and R<sup>6</sup> are as described previously, an alkylsulfonyl radical having 1 to about 8 carbon atoms; an alkylsulfonyl radical having 1 to about 6 carbon atoms substituted with cyano or hydroxy; a phenylsulfonyl radical or a phenylsulfonyl radical substituted with sulfamoyl.

phenylsulfonyl radical substituted with sulfonyl, carboxy, fluorosulfonyl or methoxy; with the proviso that there be no more than one sulfonyl radical and no more than one carboxy radical present in said compound.

47. A photosensitive element as described in claim 46 wherein

R<sup>2</sup> represents an alkylene radical having 1 to about 4 carbon atoms, phenylene or phenylene substituted with carboxy, chloro, methyl or methoxy;

L represents sulfamoyl, sulfonamido, carbamoyl, or carboxamido;

R represents hydrogen;  
 $q$  is an integer having a value of 1;  
 $m$  is an integer having a value of 0 or 1;  
Q represents hydrogen, hydroxy,  $-\text{NHCOR}^3$  or  $-\text{NHSO}_2\text{R}^3$  wherein  $\text{R}^3$  represents an alkyl radical having 1 to about 4 carbon atoms, an alkyl radical having 1 to about 4 carbon atoms substituted with hydroxy, cyano, sulfamoyl, carboxy or sulfo; benzyl, phenyl, phenyl substituted with carboxy, chloro, methyl, methoxy or sulfamoyl;

D represents chloro; fluoro; bromo; cyano; trifluoromethyl; nitro; fluorosulfonyl; alkylsulfonyl having 1 to about 6 carbon atoms; alkylsulfonyl having 1 to about 6 carbon atoms substituted with hydroxy, phenyl, cyano, sulfamoyl, carboxy or sulfo; phenylsulfonyl; phenylsulfonyl substituted with hydroxy, sulfamoyl, fluorosulfonyl, carboxy or sulfo; a sulfamoyl radical having the formula  $-\text{SO}_2\text{NHR}^6$  wherein  $\text{R}^6$  is hydrogen, an alkyl radical having 1 to about 4 carbon atoms or an alkyl radical having 1 to about 4 carbon atoms substituted with hydroxy, cyano, sulfamoyl, carboxy, or sulfo; benzyl, phenyl or phenyl substituted with hydroxy, sulfonyl, sulfamoyl, carboxy or sulfo; a carbamoyl radical having the formula  $-\text{CON}(\text{R}^5)_2$  wherein  $\text{R}^5$  is hydrogen or methyl, and

D can represent a substituent having the formula



provided that the



substituent on the naphthalene nucleus of Formula I is replaced by an M group or the



substituent on the naphthalene nucleus of Formula II is replaced by a Q group wherein Y, Ball, X, R, J, q and m are as described previously;

E represents hydrogen, fluoro or chloro; and  
M represents hydrogen or a sulfamoyl radical of the formula  $-\text{SO}_2\text{NHR}^6$  wherein  $\text{R}^6$  is hydrogen; an alkyl radical of 1 to about 4 carbon atoms; an alkyl radical having 1 to about 4 carbon atoms substituted with hydroxy, cyano, sulfamoyl, carboxy, or sulfo; benzyl, phenyl or phenyl substituted with hydroxy, sulfamoyl, carboxy or sulfo.

48. A photosensitive element as described in claim 47 wherein n and p each have a value of 0.

49. A photosensitive element as described in claim 47 wherein m has a value of 0.

50. A photosensitive element as described in claim 47 wherein G is a hydroxy radical.

51. A photosensitive element as described in claim 47 wherein E represents a hydrogen atom; and M represents a hydrogen atom.

52. A photosensitive element as described in claim 47 wherein the



containing substituent on the naphthalene nucleus is in the 5- or 6-position relative to G in Formula I and in the 5-position relative to G in Formula II;

Y represents the atoms necessary to complete a naphthalene nucleus;

$\text{R}^2$  represents an alkylene radical having 1 to about 4 carbon atoms, or phenyl;

L represents sulfamoyl or sulfonamido;

J represents sulfonyl;

Q is in the 8-position relative to G and represents hydrogen, hydroxy,  $-\text{NHSO}_2\text{CH}_3$ , or  $-\text{NHCOCH}_3$ ;

G represents hydroxy, a photographically inactive ammonium salt thereof, or a hydrolyzable acyloxy group having the formula



wherein  $\text{R}^4$  is an alkyl having 1 to about 18 carbon atoms, phenyl or phenyl substituted with chloro or nitro;

40 D represents chloro, bromo, cyano, trifluoromethyl, nitro, alkylsulfonyl having 1 to about 6 carbon atoms or benzylsulfonyl;

E represents hydrogen; and

M represents hydrogen.

53. A photosensitive element as described in claim 52 wherein X represents



G represents hydroxy or a hydrolyzable acyloxy group; and

55 D represents an alkylsulfonyl radical having 1 to about 4 carbon atoms.

54. A photosensitive element as described in claim 52 wherein -Ball is linked to the sulfonamidonaphthol nucleus through a bivalent



55. A photosensitive element as described in claim 53 wherein -Ball represents



and is in the 2-position relative to the hydroxy group.

56. A photosensitive element as described in claim 35 wherein each silver halide emulsion is a direct positive silver halide emulsion.

57. A photosensitive element as described in claim 46 wherein each silver halide emulsion is a direct positive silver halide emulsion.

58. A photographic film unit which is adapted to be processed by passing said unit between a pair of juxtaposed pressure-applying members comprising:

- a. a photosensitive element comprising a support having thereon at least one photosensitive silver halide emulsion layer and one of said layers having associated therewith a cyan image dye-providing compound;
- b. a dye image-receiving layer which is positioned on the same side of the support as the silver halide emulsion layer; and
- c. means for discharging an alkaline processing composition within said film unit; said film unit containing a silver halide developing agent and said compound having a formula as follows:



wherein

Car represents a ballasted carrier moiety which, as a function of oxidation of said compound under alkaline conditions, cleaves off from said compound releasing a diffusible dye;

X represents a bivalent linking group of the formula  $-\text{R}^2-\text{L}_n-\text{R}^2-$ , where each  $\text{R}^2$  can be the same or different and each represents an alkyne radical having 1 to about 8 carbon atoms; a phenylene radical; or a phenylene radical substituted with chloro, bromo, cyano, nitro, methoxy, methyl, carboxy or sulfo; L represents a bivalent radical selected from oxy, carbonyl, carboxamido, carbamoyl, sulfonamido, sulfamoyl, sulfinyl or sulfonyl; n is an integer having a value of 0 or 1; p is 1 when n equals 1 and p is 1 or 0 when n equals 0, provided that when p is 1 the carbon content of the sum of both  $\text{R}^2$  radicals does not exceed 14 carbon atoms;

R represents a hydrogen atom, or an alkyl radical having 1 to about 6 carbon atoms;

J represents a bivalent radical selected from sulfonyl or carbonyl;

m and q each represent an integer having a value of 0 or 1;

Q represents a hydrogen atom, a hydroxy radical or a radical having the formula  $-\text{NHCOR}^3$  or  $-\text{NHSO}_2\text{R}^3$  wherein  $\text{R}^3$  is an alkyl radical having 1 to about 6

carbon atoms, an alkyl radical having 1 to about 4 carbon atoms substituted with hydroxy, cyano, sulfamoyl, carboxy or sulfo; benzyl, phenyl, or a phenyl radical substituted with carboxy, chloro, methyl, methoxy or sulfamoyl;

G represents a hydroxy radical, a salt thereof, or a hydrolyzable acyloxy group having the formula:



wherein  $\text{R}^4$  is an alkyl radical having 1 to about 18 carbon atoms, phenyl or phenyl substituted with chloro or nitro;

D represents a halogen atom, a cyano radical, a nitro radical, a trifluoromethyl radical, an alkyl radical having 1 to about 6 carbon atoms, an alkoxy radical having 1 to about 6 carbon atoms, a carboxy radical, a carboxylic acid ester having the formula  $-\text{COOR}^4$  wherein  $\text{R}^4$  is as described previously, a fluorosulfonyl radical, a  $-\text{SO}_3-$ phenyl radical or a  $-\text{SO}_3-$ phenyl radical substituted with hydroxy, chloro, carboxy, sulfamoyl, methyl or methoxy; a sulfo radical, a sulfamoyl radical having the formula  $-\text{SO}_2\text{NR}^5\text{R}^6$  wherein  $\text{R}^5$  represents hydrogen or an alkyl group having 1 to about 6 carbon atoms and  $\text{R}^6$  represents hydrogen, an alkyl radical having 1 to about 6 carbon atoms, an alkyl radical having 1 to about 4 carbon atoms substituted with hydroxy, cyano, sulfamoyl, carboxy or sulfo; a benzyl radical, a phenyl radical, a phenyl radical substituted with hydroxy, sulfonyl, sulfamoyl, carboxy or sulfo; an alkyl carbonyl radical having 1 to about 8 carbon atoms, or a phenyl carbonyl radical, with the proviso that the carbon content of the sum of  $\text{R}^5$  and  $\text{R}^6$  not exceed 14 carbon atoms; a carbamoyl radical having the formula  $-\text{CON}(\text{R}^5)_2$ , wherein each  $\text{R}^5$  can be the same or different and is as described previously; an alkylsulfonyl radical having 1 to about 8 carbon atoms; an alkylsulfonyl radical having 1 to about 6 carbon atoms substituted with hydroxy, phenyl, cyano, sulfamoyl, carboxy or sulfo; a phenylsulfonyl radical; a phenylsulfonyl radical substituted with hydroxy, sulfonyl, sulfamoyl, carboxy or sulfo; or D can represent a substituent having the formula  $\text{Car}-[\text{X}-(\text{NR}-\text{J})_q]_m-$  or  $\text{Car}-\text{X}-\text{J}-$ , provided that the  $\text{Car}-[\text{X}-(\text{NR}-\text{J})_q]_m-$  substituent on the naphthalene nucleus of Formula I is replaced by an M group or the  $\text{Car}-\text{X}-\text{J}-\text{NH}-$  substituent on the naphthalene nucleus of Formula II is replaced by a Q group wherein Car, X, J, R, q and m are as described previously.

E represents a hydrogen atom, a halogen atom, a nitro radical, a cyano radical or a trifluoromethyl radical;

M represents a hydrogen atom, a carboxy radical, a carboxylic acid ester having the formula  $-\text{COOR}^4$  wherein  $\text{R}^4$  is as described previously, a sulfo radical, a sulfamoyl radical having the formula  $-\text{SO}_2\text{NR}^5\text{R}^6$ , a carbamoyl radical having the formula  $-\text{CON}(\text{R}^5)_2$ , wherein  $\text{R}^5$  and  $\text{R}^6$  are as described previously, an alkylsulfonyl radical having 1 to about 8 carbon atoms; an alkylsulfonyl radical having 1 to about 6 carbon atoms substituted with cyano or hydroxy; a phenylsulfonyl radical or a phenylsulfonyl radical substituted with sulfamoyl, carboxy, fluorosulfonyl or methoxy;

with the proviso that there be no more than one sulfo radical and no more than one carboxy radical present in said compound.

59. A film unit as described in claim 58 wherein n and p each have a value of 0.

60. A film unit as described in claim 58 wherein m has a value of 0.

61. A film unit as described in claim 58 wherein G is a hydroxy radical.

62. A film unit as described in claim 58 wherein E represents a hydrogen atom, a halogen atom or a nitro radical; and M represents a hydrogen atom or a sulfamoyl radical as described in claim 58.

63. The film unit of claim 58 wherein said dye image-receiving layer is located in said photosensitive element between said support and the lowermost photosensitive silver halide emulsion layer.

64. The film unit of claim 58 wherein said dye image-receiving layer is coated on a separate support and is adapted to be superimposed on said photosensitive element after exposure thereof.

65. The film unit of claim 58 wherein said discharging means is a rupturable container and is so positioned during processing of said film unit that a compressive force applied to said container by said pressure-applying members will effect a discharge, the contents of said container between said image dye-receiving layer and the layer most remote from the support of said photosensitive element.

66. The film unit of claim 58 wherein said receiving layer comprises a polymeric cationic mordant.

67. The film unit of claim 58 wherein said dye image-receiving layer comprises a polymer having units represented by the following formula in copolymerized relationship with units of at least one other ethylenically unsaturated monomer:



wherein R<sup>7</sup> and R<sup>8</sup> each represent a hydrogen atom or a lower alkyl radical and R<sup>8</sup> can additionally be a group containing at least one aromatic nucleus; Q can be a divalent alkylene radical, a divalent arylene radical, a divalent aralkylene radical, a divalent arylenealkylene radical,



wherein R<sup>12</sup> is an alkylene radical, or R<sup>8</sup> can be taken together with Q to form a



R<sup>9</sup>, R<sup>10</sup> and R<sup>11</sup> can be alkyl, aralkyl or aryl, or R<sup>9</sup> and R<sup>10</sup> and the nitrogen atom to which they are attached can together with Q represent the atoms and bonds necessary to form a quaternized nitrogen-containing heterocyclic ring, and X<sup>-</sup> is a monovalent negative

salt-forming radical or atom in ionic relationship with the positive salt-forming radical; wherein said polymer is substantially free of carboxy groups and wherein the positive salt-forming radical of said polymer comprises at least two aryl groups for each quaternary nitrogen atom in said polymer.

68. A film unit as described in claim 58 wherein R<sup>2</sup> represents an alkylene radical having 1 to about 4 carbon atoms, phenylene or phenylene substituted with carboxy, chloro, methyl or methoxy;

L represents sulfamoyl, sulfonamido, carbamoyl or carboxamido;

R represents hydrogen;

q is an integer having a value of 1;

m is an integer having a value of 0 or 1;

Q represents hydrogen, hydroxy, -NHCOR<sup>3</sup> or -NHSO<sub>2</sub>R<sup>3</sup> wherein R<sup>3</sup> represents an alkyl radical having 1 to about 4 carbon atoms; an alkyl radical having 1 to about 4 carbon atoms substituted with hydroxy, cyano, sulfamoyl, carboxy or sulfo; benzyl, phenyl or phenyl substituted with carboxy, chloro, methyl, methoxy or sulfamoyl;

D represents chloro, fluoro, bromo, cyano, trifluoromethyl, nitro, fluorosulfonyl, alkylsulfonyl having 1 to about 6 carbon atoms, alkylsulfonyl having 1 to about 6 carbon atoms substituted with hydroxy, phenyl, cyano, sulfamoyl, carboxy, or sulfo; phenylsulfonyl; phenylsulfonyl substituted with hydroxy, sulfamoyl, fluorosulfonyl, carboxy or sulfo; a sulfamoyl radical having the formula -SO<sub>2</sub>NHR<sup>6</sup> wherein R<sup>6</sup> is hydrogen, an alkyl radical having 1 to about 4 carbon atoms, or an alkyl radical having 1 to about 4 carbon atoms substituted with hydroxy, cyano, sulfamoyl, carboxy or sulfo; benzyl, phenyl or phenyl substituted with hydroxy, sulfonyl, sulfamoyl, carboxy or sulfo; a carbamoyl radical having the formula -CON(R<sup>5</sup>)<sub>2</sub> wherein R<sup>5</sup> is hydrogen or methyl, and

D can represent a substituent having the formula Car-[X-(NR-J)<sub>q</sub>]<sub>m</sub>- or Car-X-J-, provided that the Car-[X-(NR-J)<sub>q</sub>]<sub>m</sub>- substituent on the naphthalene nucleus of Formula I is replaced by an M group or the Car-X-J-NH- substituent on the naphthalene nucleus of Formula II is replaced by a Q group wherein Car, X, J, R, q and m are as described previously;

E represents hydrogen, fluoro, or chloro; and M represents hydrogen or a sulfamoyl radical of the formula -SO<sub>2</sub>NHR<sup>6</sup> wherein R<sup>6</sup> is hydrogen; an alkyl radical of 1 to about 4 carbon atoms; an alkyl radical having 1 to about 6 carbon atoms substituted with hydroxy, cyano, sulfamoyl, carboxy, or sulfo; benzyl, phenyl or phenyl substituted with hydroxy, sulfamoyl, carboxy or sulfo.

69. A film unit as described in claim 68 wherein n and p each have a value of 0.

70. A film unit as described in claim 68 wherein m has a value of 0.

71. A film unit as described in claim 68 wherein G is a hydroxy radical.

72. A film unit as described in claim 68 wherein E represents a hydrogen atom, a halogen atom or nitro radical; and M represents a hydrogen atom.

73. A film unit as described in claim 68 wherein the Car-X-J-NH-substituent in Formula II is in the 5-position on the naphthalene nucleus relative to G; and the Car-[X-(NR-J)<sub>q</sub>]<sub>m</sub>- substituent in Formula I is in the 5- or 6-position on the naphthalene nucleus relative to G;

$R^2$  represents an alkylene radical having 1 to about 4 carbon atoms, or phenylene;  
 L represents sulfamoyl or sulfonamido;  
 J represents sulfonyl;  
 Q is in the 8-position relative to G and represents hydrogen, hydroxy,  $-NHSO_2R^3$ , or  $-NHCOCH_3$ ;  
 G represents hydroxy, a photographically inactive ammonium salt thereof, or a hydrolyzable acyloxy group having the formula:

10



wherein  $R^4$  is an alkyl radical having 1 to about 18 carbon atoms, phenyl or phenyl substituted with chloro or nitro;

D represents chloro, bromo, cyano, trifluoromethyl, nitro, alkylsulfonyl having 1 to about 6 carbon atoms, or benzylsulfonyl;

E represents hydrogen; and

M represents hydrogen.

74. A film unit as described in claim 73 wherein X represents

20



G represents hydroxy or a hydrolyzable acyloxy group; and

30

D represents an alkylsulfonyl radical having 1 to about 4 carbon atoms.

75. A photographic film unit which is adapted to be processed by passing said unit between a pair of juxtaposed pressureapplying members comprising:

35

a. a photosensitive element comprising a support having thereon at least one photosensitive silver halide emulsion layer and one of said layers having associated therewith a cyan image dye-providing compound;

b. a dye image-receiving layer which is positioned on the same side of the support as the silver halide emulsion layer; and

c. means for discharging an alkaline processing composition within said film unit;

said film unit containing a silver halide developing agent and said compound having the formula as follows:

40



50



wherein

Ball represents an organic ballasting group of such size and configuration as to render said compound nondiffusible during development in an alkaline processing composition;

Y represents the carbon atoms necessary to complete a benzene or naphthalene nucleus;

X represents a bivalent linking group of the formula  $-R^2-L_n-R^2_p-$  where each  $R^2$  can be the same or different and each represents an alkylene radical having 1 to about 8 carbon atoms; a phenylene radical; or a phenylene radical substituted with chloro, bromo, cyano, nitro, methoxy, methyl, carboxy or sulfo; L represents a bivalent radical selected from oxy, carbonyl, carboxamido, carbamoyl, sulfonamido, sulfamoyl, sulfinyl or sulfonyl; n is an integer having a value of 0 or 1; p is 1 when n equals 1 and p is 1 or 0 when n equals 0, provided that when p is 1 the carbon content of the sum of both  $R^2$  radicals does not exceed 14 carbon atoms;

R represents a hydrogen atom, or an alkyl radical having 1 to about 6 carbon atoms;

J represents a bivalent radical selected from sulfonyl or carbonyl;

m and q each represent an integer having a value of 0 or 1;

Q represents a hydrogen atom, a hydroxy radical or a radical having the formula  $-NHCOR^3$  or  $-NHSO_2R^3$  wherein  $R^3$  is an alkyl radical having 1 to about 6 carbon atoms, an alkyl radical having 1 to about 4 carbon atoms substituted with hydroxy, cyano, sulfamoyl, carboxy or sulfo; benzyl, phenyl, or a phenyl radical substituted with carboxy, chloro, methyl, methoxy or sulfamoyl;

G represents a hydroxy radical, a salt thereof, or a hydrolyzable acyloxy group having the formula:



wherein  $R^4$  is an alkyl radical having 1 to about 18 carbon atoms, phenyl or phenyl substituted with chloro or nitro;

45

D represents a halogen atom, a cyano radical, a nitro radical, a trifluoromethyl radical, an alkyl radical having 1 to about 6 carbon atoms, an alkoxy radical having 1 to about 6 carbon atoms, a carboxy radical, a carboxylic acid ester having the formula  $-COOR^4$  wherein  $R^4$  is as described previously, a fluorosulfonyl radical, a  $-SO_3-$ phenyl radical or a  $-SO_3-$ phenyl radical substituted with hydroxy, chloro, carboxy, sulfamoyl, methyl or methoxy; a sulfo radical, a sulfamoyl radical having the formula  $-SO_2NR^5R^6$  wherein  $R^5$  represents hydrogen or an alkyl group having 1 to about 6 carbon atoms and  $R^6$  represents hydrogen, an alkyl radical having 1 to about 6 carbon atoms, an alkyl radical having 1 to about 4 carbon atoms substituted with hydroxy, cyano, sulfamoyl, carboxy or sulfo; a benzyl radical, a phenyl radical, a phenyl radical substituted with hydroxy, sulfonamido, sulfamoyl, carboxy or sulfo; an alkyl carbonyl radical having 1 to about 8 carbon atoms, or a phenyl carbonyl radical, with the proviso that the carbon content of the sum of  $R^5$  and  $R^6$  not exceed 14 carbon atoms; a carbamoyl radical of the formula  $-CON(R^5)_2$  wherein each  $R^5$  can be the same or different and is as described

previously; an alkylsulfonyl radical having 1 to about 8 carbon atoms; an alkylsulfonyl radical having 1 to about 6 carbon atoms substituted with hydroxy, phenyl, cyano, sulfamoyl, carboxy or sulfo; a phenylsulfonyl radical; a phenylsulfonyl radical substituted with hydroxy, sulfonyl, sulfamoyl, carboxy or sulfo; or D can represent a substituent having the formula



provided that the



substituent on the naphthalene nucleus of Formula I is replaced by an M group or the



substituent on the naphthalene nucleus of formula II is replaced by a Q group wherein Car, X, J, R, q and m are as described previously.

E represents a hydrogen atom, a halogen atom, a nitro radical, a cyano radical or a trifluoromethyl radical;

M represents a hydrogen atom, a carboxy radical, a carboxylic acid ester having the formula -COOR<sup>4</sup> wherein R<sup>4</sup> is as described previously, a sulfo radical, a sulfamoyl radical having the formula -SO<sub>2</sub>NR<sup>5</sup>R<sup>6</sup>, a carbamoyl radical having the formula -CON(R<sup>5</sup>)<sub>2</sub> wherein R<sup>5</sup> and R<sup>6</sup> are as described previously, an alkylsulfonyl radical having 1 to about 8 carbon atoms; an alkylsulfonyl radical having 1 to about 6 carbon atoms substituted with cyano or hydroxy; a phenylsulfonyl radical or a phenylsulfonyl radical substituted with sulfamoyl, carboxy, fluorosulfonyl or methoxy;

with the proviso that there be no more than one sulfo radical and no more than one carboxy radical present in said compound.

76. The film unit of claim 75 wherein said dye image-receiving layer is located in said photosensitive element between said support and the lowermost photosensitive silver halide emulsion layer.

77. The film unit of claim 75 wherein said dye image-receiving layer is coated on a separate support and is adapted to be superimposed on said photosensitive element after exposure thereof.

78. The film unit of claim 75 wherein said discharging means is a rupturable container and is so positioned during processing of said film unit that a compressive force applied to said container by said pressure-applying

10



will effect a discharge, the contents of said container between said image dye-receiving layer and the layer most remote from the support of said photosensitive element.

79. The film unit of claim 75 wherein said receiving layer comprises a polymer cationic mordant.

80. A film unit of claim 75 wherein said dye image-receiving layer comprises a polymer having units represented by the following formula in copolymerized relationship with units of at least one other ethylenically unsaturated monomer:

wherein R<sup>7</sup> and R<sup>8</sup> each represent a hydrogen atom or a lower alkyl radical and R<sup>8</sup> can additionally be a group containing at least one aromatic nucleus; Q can be a divalent alkylene radical, a divalent arylene radical, a divalent aralkylene radical, a divalent arylenealkylene radical,

35



wherein R<sup>12</sup> is an alkylene radical, or R<sup>8</sup> can be taken together with Q to form a



group; R<sup>9</sup>, R<sup>10</sup> and R<sup>11</sup> can be alkyl, aralkyl or aryl, or R<sup>9</sup> and R<sup>10</sup> and the nitrogen atom to which they are attached can together with Q represent the atoms and bonds necessary to form a quaternized nitrogen-containing heterocyclic ring, and X<sup>-</sup> is a monovalent negative salt-forming radical or atom in ionic relationship with the positive salt-forming radical or atom in said polymer is substantially free of carboxy groups and wherein the positive salt-forming radical of said polymer comprises at least two aryl groups for each quaternary nitrogen atom in said polymer.

81. A film unit as described in claim 75 wherein R<sup>2</sup> represents an alkylene radical having 1 to about 4 carbon atoms, phenylene or phenoxy substituted with carboxy, chloro, methyl or methoxy;

L represents sulfamoyl, sulfonamido, carbamoyl or carboxamido;

R represents hydrogen;

q is an integer having a value of 1;

m is an integer having a value of 0 or 1;

Q represents hydrogen, hydroxy, -NHCOR<sup>3</sup> or -NHSO<sub>2</sub>R<sup>3</sup> wherein R<sup>3</sup> represents an alkyl radical

having 1 to about 4 carbon atoms, an alkyl radical having 1 to about 4 carbon atoms substituted with hydroxy, cyano, sulfamoyl, carboxy or sulfo; benzyl, phenyl, phenyl substituted with carboxy, chloro, methyl, methoxy or sulfamoyl;

D represents chloro; fluoro; bromo; cyano; trifluoromethyl; nitro; fluorosulfonyl; alkylsulfonyl having 1 to about 6 carbon atoms; alkylsulfonyl having 1 to about 6 carbon atoms substituted with hydroxy, phenyl, cyano, sulfamoyl, carboxy or sulfo; phenylsulfonyl; phenylsulfonyl substituted with hydroxy, sulfamoyl, fluorosulfonyl, carboxy or sulfo; a sulfamoyl radical having the formula  $-\text{SO}_2\text{NHR}^6$  wherein  $\text{R}^6$  is hydrogen, an alkyl radical having 1 to about 4 carbon atoms or an alkyl radical having 1 to about 4 carbon atoms substituted with hydroxy, cyano, sulfamoyl, carboxy, or sulfo; benzyl, phenyl or phenyl substituted with hydroxy, sulfonyl, sulfamoyl, carboxy or sulfo; a carbamoyl radical having the formula  $-\text{CON}(\text{R}^5)_2$  wherein  $\text{R}^5$  is hydrogen or methyl, and D can represent a substituent having the formula



provided that the



substituent on the naphthalene nucleus of Formula I is replaced by an M group or the



substituent on the naphthalene nucleus of Formula II is replaced by a Q group wherein Y, Ball, X, R, J, q and m are as described previously;

E represents hydrogen, fluoro or chloro; and M represents hydrogen or a sulfamoyl radical of the formula  $-\text{SO}_2\text{NHR}^6$  wherein  $\text{R}^6$  is hydrogen; an alkyl radical of 1 to about 4 carbon atoms; an alkyl radical having 1 to about 4 carbon atoms substituted with hydroxy, cyano, sulfamoyl, carboxy, or sulfo; benzyl, phenyl or phenyl substituted with hydroxy, sulfamoyl, carboxy or sulfo.

82. A film unit as described in claim 81 wherein n and p each have a value of 0.

83. A film unit as described in claim 81 wherein m has a value of 0.

84. A film unit as described in claim 81 wherein G is a hydroxy radical.

85. A film unit as described in claim 81 wherein E represents a hydrogen atom; and M represents a hydrogen atom.

86. A film unit as described in claim 81 wherein the



containing substituent on the naphthalene nucleus is in the 5- or 6-position relative to G in Formula I and in the 5-position relative to G in Formula II;

Y represents the atoms necessary to complete a naphthalene nucleus;

$\text{R}^2$  represents an alkylene radical having 1 to about 4 carbon atoms, or phenyl;

L represents sulfamoyl or sulfonamido;

J represents sulfonyl;

Q is in the 8-position relative to G and represents hydrogen, hydroxy,  $-\text{NHSO}_2\text{CH}_3$ , or  $-\text{NHCOCH}_3$ ;

G represents hydroxy, a photographically inactive ammonium salt thereof, or a hydrolyzable acyloxy group having the formula



wherein  $\text{R}^4$  is an alkyl having 1 to about 18 carbon atoms, phenyl or phenyl substituted with chloro or nitro;

D represents chloro, bromo, cyano, trifluoromethyl, nitro, alkylsulfonyl having 1 to about 6 carbon atoms or benzylsulfonyl;

E represents hydrogen; and

M represents hydrogen.

87. A film unit as described in claim 86 wherein X represents



50 G represents hydroxy or a hydrolyzable acyloxy group; and

D represents an alkylsulfonyl radical having 1 to about 4 carbon atoms.

88. A film unit as described in claim 86 wherein -Ball is linked to the sulfonamidonaphthol nucleus through a bivalent



moiety.

89. A film unit as described in claim 87 wherein -Ball represents



and is in the 2-position relative to the hydroxy group.

90. A photosensitive element as described in claim 12 wherein X represents



E represents hydroxy and D represents methylsulfonyl.

91. A photosensitive element as described in claim 22 wherein X represents



G represents hydroxy and D represents methylsulfonyl.

92. A photosensitive element as described in claim 20 wherein -Ball represents



and is in the 2-position relative to the hydroxy group.

93. A photosensitive element as described in claim 19 wherein -Ball represents



and is in the 2-position relative to the hydroxy group.

94. A photosensitive element as described in claim 92 wherein X represents

10



15 G represents hydroxy, and D represents methylsulfonyl.

95. A photosensitive element as described in claim 91 wherein said cyan image dye-providing compound is contained in a layer contiguous to the silver halide emulsion layer.

96. A photosensitive element as described in claim 93 wherein said cyan image dye-providing compound is contained in a layer contiguous to the silver halide emulsion layer.

97. A photosensitive element as described in claim 95 wherein each silver halide emulsion is a direct positive silver halide emulsion.

98. A photosensitive element as described in claim 96 wherein each silver halide emulsion is a direct positive silver halide emulsion.

\* \* \* \* \*

35

40

45

50

55

60

65